



US006258494B1

(12) **United States Patent**  
Bourdelais et al.

(10) **Patent No.:** US 6,258,494 B1  
(45) **Date of Patent:** Jul. 10, 2001

(54) **DUPLITIZED PHOTOGRAPHIC DEPTH IMAGING**

(75) Inventors: **Robert P. Bourdelais**, Pittsford; **Peter T. Aylward**, Hilton; **Alphonse D. Camp**, Rochester, all of NY (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **09/470,240**

(22) Filed: **Dec. 22, 1999**

(51) **Int. Cl.<sup>7</sup>** ..... **G03C 1/46**; G03C 1/77; G03C 1/775; G03C 11/14

(52) **U.S. Cl.** ..... **430/15**; 430/502; 430/506; 430/536; 430/538; 430/952; 430/432

(58) **Field of Search** ..... 430/15, 502, 261, 430/952, 536, 538, 432, 506

(56) **References Cited**

U.S. PATENT DOCUMENTS

2,887,379 \* 5/1959 Blake et al. ..... 430/538

|           |           |                                 |
|-----------|-----------|---------------------------------|
| 4,040,830 | 9/1977    | Rogers .                        |
| 4,355,099 | * 10/1982 | Trautweiler ..... 430/538       |
| 4,629,667 | 12/1986   | Kistner et al. ..... 430/11     |
| 5,424,175 | 6/1995    | Ueda et al. ..... 430/403       |
| 5,449,597 | * 9/1995  | Sawyer ..... 430/523            |
| 5,639,580 | 6/1997    | Morton ..... 430/11             |
| 5,681,676 | 10/1997   | Telfer et al. ..... 430/22      |
| 5,744,291 | 4/1998    | Ip ..... 430/504                |
| 5,866,282 | 2/1999    | Bourdelais et al. ..... 430/538 |
| 6,017,685 | 1/2000    | Bourdelais et al. ..... 430/536 |
| 6,030,742 | 2/2000    | Bourdelais et al. ..... 430/536 |
| 6,030,756 | 2/2000    | Bourdelais et al. ..... 430/536 |
| 6,071,654 | * 6/2000  | Camp et al. ..... 430/536       |
| 6,080,532 | * 6/2000  | Camp et al. ..... 430/536       |

\* cited by examiner

*Primary Examiner*—Richard L. Schilling

(74) *Attorney, Agent, or Firm*—Paul A. Leipold

(57) **ABSTRACT**

This invention relates to a photographic element comprising a transparent sheet having a developed photographic image on each side, adhesively connected to a reflective base.

**61 Claims, No Drawings**

## 1

DUPLICITIZED PHOTOGRAPHIC DEPTH  
IMAGING

## FIELD OF THE INVENTION

This invention relates to photographic materials. In a preferred form it relates to a photographic reflective images.

## BACKGROUND OF THE INVENTION

In the formation of color paper it is known that the base paper has applied thereto a layer of polymer, typically polyethylene. This layer serves to provide waterproofing to the paper, as well as providing a smooth surface on which the photosensitive layers are formed. The formation of a suitably smooth surface is difficult requiring great care and expense to ensure proper lay down and cooling of the polyethylene layers. The formation of a suitably smooth surface would improve image quality as the display material would have more apparent blackness as the reflective properties of the improved base are more specular than the prior materials. As the whites are whiter and the blacks are blacker, there is more range in between and, therefore, contrast is enhanced. It would be desirable if a more reliable and smoother surface could be formed at less expense.

Prior art photographic reflective papers are typically coated with silver halide imaging layers that contain a separate layer for the magenta, cyan and yellow layers. The color coupler containing layers are typically separated by gelatin inter layers that provide spacing. The spacing of the color coupler containing layers with gelatin inter layers creates a sense of depth in the image to the observer. This sense of depth adds to the quality of a silver halide image and perceptually differentiates a silver halide image from imaging techniques that are more planar. For example, ink jet images do not typically have separation between the ink drops that make up an ink jet image and thus ink jet images appear flat and some what lifeless compared to the same image created from silver halide imaging layers.

It has been found that by increasing the thickness of the gelatin inter layers that the depth of image for a silver halide image can be improved. However, increasing the thickness of the gelatin inter layers reduces the efficiency of the image development process and increases the cost of the imaging material. Also, by increasing the thickness of the gelatin inter layer, the yellowness of the imaging layers causes the density minimum areas to appear more yellow which is undesirable as consumers perceptually prefer density minimum areas that have a slight blue tint.

Prior art stereo photography or depth photography uses visual simulation to provide photographs that can be seen in three dimensions. A stereo camera has two lens placed about 65 mm apart, which is the average interpupillary distance for adults. Two photographs are taken simultaneously of the subject. A stereo viewer is used to present the photograph taken by the left lens to the left eye simultaneously with the one taken by the right lens to the right eye. The human brain then fuses the images into a single image and a three dimensional image of the original subject is seen.

It has been proposed in U.S. Pat. No. 5,866,282 Bourdeais et al. to utilize a composite support material with laminated biaxially oriented polyolefin sheets as a photographic imaging material. In U.S. Pat. No. 5,866,282 biaxially oriented polyolefin sheets are extrusion laminated to cellulose paper to create a support for silver halide imaging layers. The biaxially oriented sheets described in U.S. Pat. No. 5,866,282 have a microvoided layer in combination with coextruded layers that contain white pigments. The

## 2

composite imaging support structure described in U.S. Pat. No. 5,866,282 has been found to be more durable, sharper and brighter than prior art photographic paper imaging supports that use cast melt extruded polyethylene layers coated on cellulose paper.

Typically, photographic reflective imaging layers are coated on a polyethylene coated cellulose paper. While polyethylene coated cellulose paper does provide an acceptable support for the imaging layers, there is a need for alternate support materials such as polyester or fabric. The problem with alternate, non paper supports is the lack of robustness in photographic processing equipment to mechanical property changes in supports. The photographic processing equipment will not run photographic materials that have significantly different mechanical properties than prior art photographic materials. It would be desirable if a reflective photographic image could be efficiently formed on alternate supports.

The continuing thrust towards digital printing of photographic color papers has created the need for color imaging materials that can work in both a negative working optical and digital exposure equipment. In order for color silver halide imaging materials to correctly print digitally, a color negative curve shape of the imaging material is critical. In a digital environment (direct writing) to a photographic paper, the curve shape to a degree can be electromodulated and thus have a greater degree of freedom that the optical printing of the color negative working system. Ideally, a color paper type imaging system that could substantially maintain tone scale from conventional optical negative working exposure times to sub microsecond digital direct writing exposure times would be preferred. This would enable a photofinishing area to maintain one material for both digital and optical exposure thereby reducing the need for expensive inventory.

PROBLEM TO BE SOLVED BY THE  
INVENTION

There is a continuing need for silver halide images that have improved depth of image. Further, there is also continuing need for photographic elements that are more durable in use and lighter weight for handling during the formation, imaging, and development process.

## SUMMARY OF THE INVENTION

It is an object of the invention to overcome disadvantages of prior photographic elements.

It is another object of the invention to provide a silver halide image with improved image depth properties.

It is another object to provide photographic elements that are lightweight and thin.

It is a further object to provide photographic elements that may be easily provided in finished form with a variety of substrates.

These and other objects of the invention are accomplished by a photographic element comprising a transparent sheet having a developed photographic image on each side, adhesively connected to a reflective base.

ADVANTAGEOUS EFFECT OF THE  
INVENTION

The invention provides a photographic element that is has an improved sense of depth, light in weight for ease of formation, imaging and development but may be easily adhered to a variety of substrates.

## DETAILED DESCRIPTION OF THE INVENTION

The invention has numerous advantages over prior photographic elements. The elements of the invention convey a greater sense of image depth than prior art materials. This is especially attractive for consumer images as typical consumer image content often contain both foreground and background content. Images with a greater sense of depth better recall the event, time and place that the image was captured as it provides an image with three dimensional qualities. Further, photography and digital display media such as television has traditionally been a two dimensional representation of the three dimensional world. Depth of image has been shown to be perceptually preferred representation of the world.

The elements of the invention are also lighter in weight and thickness so that a roll of the photographic element of the same diameter will contain many more linear feet resulting in many more images per roll. The imaging element of the invention after development may be easily adhered to a variety of substrates, thereby allowing customized use of the images. It may be desirable for images that will be mailed, to be adhered to a lightweight substrate, whereas images to be displayed can easily be adhered to a heavy substrate after their development. The base material that is utilized in mounting of the photographic images of the invention may be lower in cost, as it is not present during development of the image and not subjected to the development chemicals. The problem of dusting during slitting and chopping of photographic elements is greater minimized, as slitting and chopping takes place when there is no base substrate present. These and other advantages will be apparent from the detailed description below.

The term as used herein, "transparent" means the ability to pass radiation without significant deviation or absorption. For this invention, "transparent" material is defined as a material that has a spectral transmission greater than 90%. For a photographic element, spectral transmission is the ratio of the transmitted power to the incident power and is expressed as a percentage as follows;  $T_{RGB}=10^{-D} * 100$  where D is the average of the red, green and blue Status A transmission density response measured by an X-Rite model 310 (or comparable) photographic transmission densitometer. For this invention, "reflective" print material is defined as a print material that has a spectral transmission of 15% or less.

The term as used herein, "foreground" means the silver halide imaging layers that are exposed after the transparent sheet of the invention has been laminated to the base. The term as used herein, "background" means the silver halide imaging layers that are encapsulated between the transparent sheet and the base utilized in the invention after post image development lamination.

For the photographic element of this invention the light sensitive silver halide imaging layers are coated onto both sides of a thin polymer sheet that contains an emulsion adhesion layer on each side. The silver halide imaging layers on each side of the thin polymer sheet are then be simultaneously exposed on each side with images using conventional negative working optical exposure technology or digital exposure devices so that the exposed imaging layers are in registration. The polymer sheet with the printed imaging layers of each side is subsequently processed using traditional photographic chemistry. When the thin transparent biaxially oriented sheet with the developed images are adhered to a reflective base material with the image, a

photographic reflective print material is created that has an improved sense of image depth. Since an image with an improved sense of depth is a better representation of reality, it has significant consumer value compared to flat images that are common to ink jet printed images.

Because the light sensitive imaging layers that are applied to each side of the transparent sheet are imaged simultaneously, the registration of the image from the foreground to the background is exact. This quality of registration obtained in this invention is critical for the formation of a realistic and believable depth image. Since the silver halide imaging layers are exposed and processed without a base material, it was discovered that image sharpness of the image is exceptional, far exceeding the image sharpness of images printed on photographic paper.

The silver halide image layers are applied to both sides of the transparent polymer sheet. Applying typical imaging layer thickness to both sides of the transparent polymer yielded images that were dark and did not show much depth of image improvement compared to prior art photographic paper. Reducing the silver halide imaging layer coverage to approximately 50% on each side created a quality image with a improved sense of depth. Additionally, by reducing the silver halide coverage on both sides, the development time for the image was also reduced. Reducing image development time has significant commercial value to photographic processors as the efficiency of the processing operation can be improved.

The thickness and the optical transmission of the transparent sheet of the invention are critical to the performance of the silver halide depth image. For the transparent sheet of the invention, an optical transmission of greater than 90% is preferred. An optical transmission of the transparent sheet less than 88% begins to degrade the quality of the background image thus decreasing the quality the depth image. The transparent sheet thickness determines the amount of depth that the image contains. The preferred thickness of the transparent sheet is between 6 and 100 micrometers. Below 4 micrometers the sheet is difficult to transport in manufacturing and photographic processing. Above 125 micrometers, the quality of the image begins to degrade during off angle viewing when the image begins to appear out of register.

The transparent sheet is thin, preferably less than 100 micrometers. A thin transparent sheet has the advantage of allowing longer rolls of light sensitive silver halide coated rolls compared with thick cellulose paper based utilized in prior art materials. The thin polymer sheets also significantly reduce shipping cost of developed images as the thin biaxially oriented polymer sheet of the invention weight significantly less than prior art photographic paper. A thin sheet is also necessary to reduce unwanted reduction in the transparency of the biaxially oriented sheet resulting in a cloudy image as the thin biaxially oriented sheet is laminated to a reflective support.

Another unique feature of this invention is the addition of an antihalation layer to the background imaging layer. The antihalation layer prevents unwanted secondary exposure of the silver crystals in the imaging layer as light is absorbed in the antihalation layer during exposure. The prevention of secondary exposure of the light sensitive silver crystals, will significantly increase the sharpness of the image without the use of  $TiO_2$  which is commonly used in prior art reflective photographic print materials. The antihalation is removed during development.

Surprisingly, it has also been found that polymer chemistry can be added to the transparent sheet to provide

ultraviolet protection to the couplers used in the background image layers. Traditionally, ultraviolet radiation protection for prior art reflective materials has been provided in a gelatin overcoat layer. The incorporation of the ultraviolet protection materials in the polymer sheet of this invention provides better ultraviolet protection to the imaging couplers and is lower in cost as less ultraviolet filter materials are required in the polymer transparent sheet than in a gelatin overcoat.

By printing and developing the image on the transparent sheet and then laminating to a reflective base, this invention avoids many of the problems associated with coating the light sensitive emulsions on to a base material. For example, problems such as paper dusting during slitting and punching, edge penetration of processing chemicals into the exposed paper along the slit edge and unwanted secondary reflection caused by the paper base. Further, for prior art photographic reflective print materials, great care must be taken to ensure that the paper base does not chemically sensitize the light sensitive image layers prior to processing. By joining the imaging layers with a reflective base after processing, a lower cost base can be used because the base material could not interact with the sensitized layers. Joining of the imaging layers of this invention with a reflective base after processing would allow many different types of base materials to be used, offering the consumer a range of options such as paper, polymer base or fabric base.

Suitable thin, transparent sheets for the coating of the silver halide imaging must not interfere with the light sensitive silver halide imaging layers utilized in this invention. Further the transparent sheet needs to be flexible and tough to withstand the rigors of high speed packaging equipment and handling of the package by retailers and consumers. Biaxially oriented polymer sheets are preferred and manufactured by coextrusion of the sheet, which may contain several layers, followed by biaxial orientation. Such biaxially oriented sheets are disclosed in, for example, U.S. Pat. No. 4,764,425. Biaxially oriented sheet are preferred as the orientation process produces a thin, tough transparent polymer sheet that has an acceptable surface for the application of silver halide imaging layers.

Preferred classes of thermoplastic polymers for the transparent sheet include polyolefins, polyesters, polyamides, polycarbonates, cellulosic esters, polystyrene, polyvinyl resins, polysulfonamides, polyethers, polyimides, polyvinylidene fluoride, polyurethanes, polyphenylenesulfides, polytetrafluoroethylene, polyacetals, polysulfonates, polyester ionomers, and polyolefin ionomers. Copolymers and/or mixtures of these polymers can be used.

Polyolefins particularly polypropylene, polyethylene, polymethylpentene, and mixtures thereof are preferred for the transparent sheet. Polyolefin copolymers, including copolymers of propylene and ethylene such as hexene, butene and octene are also preferred. Polypropylenes are most preferred because they are low in cost and have good strength and surface properties.

Preferred polyesters for the transparent sheet of the invention include those produced from aromatic, aliphatic or cycloaliphatic dicarboxylic acids of 4-20 carbon atoms and aliphatic or alicyclic glycols having from 2-24 carbon atoms. Examples of suitable dicarboxylic acids include terephthalic, isophthalic, phthalic, naphthalene dicarboxylic acid, succinic, glutaric, adipic, azelaic, sebacic, fumaric, maleic, itaconic, 1,4-cyclohexanedicarboxylic, sodiosulfosophthalic and mixtures thereof. Examples of suitable glycols include ethylene glycol, propylene glycol,

butanediol, pentanediol, hexanediol, 1,4-cyclohexanediethanol, diethylene glycol, other polyethylene glycols and mixtures thereof. Such polyesters are well known in the art and may be produced by well known techniques, e.g., those described in U.S. Pat. No. 2,465,319 and U.S. Pat. No. 2,901,466. Preferred continuous matrix polyesters are those having repeat units from terephthalic acid or naphthalene dicarboxylic acid and at least one glycol selected from ethylene glycol, 1,4-butanediol and 1,4-cyclohexanediethanol. Poly(ethylene terephthalate), which may be modified by small amounts of other monomers, is especially preferred. Other suitable polyesters include liquid crystal copolymers formed by the inclusion of suitable amount of a co-acid component such as stilbene dicarboxylic acid. Examples of such liquid crystal copolymers are those disclosed in U.S. Pat. Nos. 4,420,607; 4,459,402; and 4,468,510.

Useful polyamides for the transparent sheet include nylon 6, nylon 66, and mixtures thereof. Copolymers of polyamides are also suitable continuous phase polymers. An example of a useful polycarbonate is bisphenol-A polycarbonate. Cellulosic esters suitable for use as the continuous phase polymer of the composite sheets include cellulose nitrate, cellulose triacetate, cellulose diacetate, cellulose acetate propionate, cellulose acetate butyrate, and mixtures or copolymers thereof. Useful polyvinyl resins include polyvinyl chloride, poly(vinyl acetal), and mixtures thereof. Copolymers of vinyl resins can also be utilized.

The transparent sheet of the invention preferably contains a silver halide adhesion layer on each side. A silver halide adhesion layer is one that promotes adhesion between the transparent sheet and the silver halide emulsions typically containing gelatin. The transparent sheet would have coatings applied to both sides on the transparent sheet if needed. If one or both surface layers of the transparent support sheet comprise polyethylene, then there is less need for the silver halide adhesion layer. Subbing layers used to promote adhesion of coating compositions to the support are well known in the art and any such material can be employed. Some useful compositions for this purpose include interpolymers of vinylidene chloride such as vinylidene chloride/methyl acrylate/itaconic acid terpolymers or vinylidene chloride/acrylonitrile/acrylic acid terpolymers, and the like. These and other suitable compositions are described, for example, in U.S. Pat. Nos. 2,627,088; 2,698,240; 2,943,937; 3,143,421; 3,201,249; 3,271,178; 3,443,950; 3,501,301. The polymeric subbing layer is usually overcoated with a second subbing layer comprised of gelatin, typically referred to as gel sub.

In a preferred embodiment of the invention, the transparent sheet is provided with an integral emulsion adhesion layer. The total thickness of the top most skin layer or exposed surface layer should be between 0.20 micrometers and 1.5 micrometers, preferably between 0.5 and 1.0 micrometers. Below 0.5 micrometers any inherent non-planarity in the coextruded skin layer may result in unacceptable color variation. At skin thickness greater than 1.0 micrometers, there is little benefit in the photographic optical properties such as image resolution. At thickness greater than 1.0 micrometers there is also a greater material volume to filter for contamination such as clumps, poor color pigment dispersion, or contamination.

Addenda may be added to the transparent sheet to change the color of the imaging element. For a photographic label, a transparent polymer sheet with a slight bluish tinge is preferred. The addition of the slight bluish tinge may be accomplished by any process which is known in the art

including the machine blending of color concentrate prior to extrusion and the melt extrusion of blue colorants that have been pre-blended at the desired blend ratio. Colored pigments that can resist extrusion temperatures greater than 320° C. are preferred as temperatures greater than 320° C. are necessary for coextrusion of the skin layer. Blue colorants used in this invention may be any colorant that does not have an adverse impact on the imaging element. Preferred blue colorants include Phthalocyanine blue pigments, Cromophthal blue pigments, Irgazin blue pigments, Irgalite organic blue pigments and pigment Blue 60.

The preferred integral emulsion adhesion layer for the transparent sheet is polyethylene. Polyethylene is relatively easy to coextrude and orient. Gelatin based light sensitive silver halide imaging layers also adhere well to polyethylene after a corona discharge treatment prior to emulsion coating. This avoids the need for expensive emulsion adhesion promoting coating being applied to obtain acceptable emulsion adhesion between the biaxially oriented sheets of this invention and the image forming layers.

The refractive index of the transparent sheet is an important characteristic that determines the extent of the depth silver halide image and the quality of the image. The reflective index of the transparent sheet is the change in direction of a light ray passing from one medium to another of different density. The ratio of the sine of the angle of incidence to the sine of the angle of refraction is defined as the index of refraction. The index of refraction may also be defined as the ratio of the velocity of light in a vacuum to the velocity of light in the transparent sheet. To optimize the depth of image for the silver halide imaging layers coated on both sides of the transparent sheet both the thickness of the transparent sheet and the index of refraction must be considered. The preferred ratio of the thickness of the transparent sheet (measured in micrometers) to the index of refraction of the transparent sheet is between 4 and 55.

Suitable base sheets for lamination to the silver halide imaging layers needs to be tough and reflective to provide an acceptable reflective depth image. Biaxially oriented polymer sheets and composite structures utilizing biaxially oriented sheet, such as the base structure disclosed in U.S. Pat. No. 5,866,282 (Bourdelaix et al) have been shown to provide both toughness and a highly reflective surface. Biaxially oriented polymer sheets are preferred and manufactured by coextrusion of the sheet, which may contain several layers, followed by biaxial orientation. Such biaxially oriented sheets are disclosed in, for example, U.S. Pat. No. 4,764,425. Biaxially oriented sheets are preferred as the orientation process produces a thin, tough transparent polymer sheet that has the required mechanical characteristic to withstand the rigors of a high speed packaging equipment.

Preferred classes of thermoplastic polymers for the base sheet include polyolefins, polyesters, polyamides, polycarbonates, cellulosic esters, polystyrene, polyvinyl resins, polysulfonamides, polyethers, polyimides, polyvinylidene fluoride, polyurethanes, polyphenylenesulfides, polytetrafluoroethylene, polyacetals, polysulfonates, polystyrene ionomers, and polyolefin ionomers. Copolymers and/or mixtures of these polymers can be used.

Polyolefins particularly polypropylene, polyethylene, polymethylpentene, and mixtures thereof are preferred for the flexible, tough polymer sheet. Polyolefin copolymers, including copolymers of propylene and ethylene such as hexene, butene and octene are also preferred. Polypropylenes are most preferred because they are low in cost and have good strength and surface properties.

Preferred polyesters for the base sheet of the invention include those produced from aromatic, aliphatic or cycloaliphatic dicarboxylic acids of 4-20 carbon atoms and aliphatic or alicyclic glycols having from 2-24 carbon atoms. Examples of suitable dicarboxylic acids include terephthalic, isophthalic, phthalic, naphthalene dicarboxylic acid, succinic, glutaric, adipic, azelaic, sebacic, fumaric, maleic, itaconic, 1,4-cyclohexanedicarboxylic, sodiosulfosiphthalic and mixtures thereof. Examples of suitable glycols include ethylene glycol, propylene glycol, butanediol, pentanediol, hexanediol, 1,4-cyclohexanenedimethanol, diethylene glycol, other polyethylene glycols, and mixtures thereof. Such polyesters are well known in the art and may be produced by well known techniques, e.g., those described in U.S. Pat. No. 2,465,319 and U.S. Pat. No. 2,901,466. Preferred continuous matrix polyesters are those having repeat units from terephthalic acid or naphthalene dicarboxylic acid and at least one glycol selected from ethylene glycol, 1,4-butanediol and 1,4-cyclohexanenedimethanol. Poly(ethylene terephthalate), which may be modified by small amounts of other monomers, is especially preferred. Other suitable polyesters include liquid crystal copolymers formed by the inclusion of suitable amount of a co-acid component such as stilbene dicarboxylic acid. Examples of such liquid crystal copolymers are those disclosed in U.S. Pat. Nos. 4,420,607, 4,459,402 and 4,468,510.

Useful polyamides for base sheet include nylon 6, nylon 66, and mixtures thereof. Copolymers of polyamides are also suitable continuous phase polymers. An example of a useful polycarbonate is bisphenol-A polycarbonate. Cellulosic esters suitable for use as the continuous phase polymer of the composite sheets include cellulose nitrate, cellulose triacetate, cellulose diacetate, cellulose acetate propionate, cellulose acetate butyrate, and mixtures or copolymers thereof. Useful polyvinyl resins include polyvinyl chloride, poly(vinyl acetal), and mixtures thereof. Copolymers of vinyl resins can also be utilized.

Addenda are preferably added to the base sheet to improve the whiteness of these sheets. This would include any process which is known in the art including adding a white pigment, such as titanium dioxide, barium sulfate, clay, or calcium carbonate. This would also include adding fluorescing agents which absorb energy in the ultraviolet region and emit light largely in the blue region, or other additives which would improve the physical properties of the sheet or the manufacturability of the sheet.

Microvoided polymer sheets are preferred as microvoided sheets have been shown to improve image whiteness without the expensive need for high percent additions of white pigments. "Void" is used herein to mean devoid of added solid and liquid matter, although it is likely the "voids" contain gas. The void-initiating particles which remain in the finished packaging sheet core should be from 0.1 to 10  $\mu\text{m}$  in diameter and preferably round in shape to produce voids of the desired shape and size. The size of the void is also dependent on the degree of orientation in the machine and transverse directions. Ideally, the void would assume a shape which is defined by two opposed and edge contacting concave disks. In other words, the voids tend to have a lens-like or biconvex shape. The voids are oriented so that the two major dimensions are aligned with the machine and transverse directions of the sheet. The Z-direction axis is a minor dimension and is roughly the size of the cross diameter of the voiding particle. The voids generally tend to be closed cells, and thus there is virtually no path open from one side of the voided-core to the other side through which gas or liquid can traverse.

The preferred thickness of the base sheet is less than 100 micrometers. The most preferred thickness of the base polymer sheet is between 20 and 80 micrometers. At a base thickness less than 15 micrometers it is difficult to provide required reflection properties for the base sheet. At thickness greater than 100 micrometers, little improvement in image optical properties such as image sharpness and lightness has been observed.

For a white, reflective depth image, the preferred optical transmission of the base polymer sheet is less than 15%. It has been found that polymer sheets with optical transmission greater than 20% have density minimum areas of the print that appear dark. Also, a base material with an optical transmission greater than 20% begins to suffer from back side show though as images are viewed by consumers. The preferred L\* of the white, reflective base material is at least 93.5. Below 93.0, the density minimum areas of the depth silver halide images will appear dark and less desirable. L\* or lightness is measured using a Spectrogard spectrophotometer, CIE system, using illuminant D6500.

The preferred percent light reflection for the base material of the invention between 400 and 700 nm is at least 90%. A percent reflection less than 87% has been shown to begin to degrade the quality of the image. Further, any wave length of light between 400 and 700 that does not have at least a 90% reflection will contain unwanted absorption that an impact the quality of the depth image.

The base material is preferably retro reflective, that is the base has the optical property of reflecting incident light energy back in the same direction from which the light energy came. A preferred retro reflective base is one that contains many tiny 90 degree prism corner reflectors formed in the surface of the base material to be laminated to the back ground silver halide imaging layers. The density of the 90 degree prism corner reflectors preferably is between 0.2 prisms/mm and 10 prisms/mm. Below 0.10 prisms/mm, the surface does not appear acceptably retro reflective. Above 12 prisms/mm, the additional cost is not justified. Another preferred retro reflective base is one that contains precision ground glass that reflects incident light energy back in the same direction from which the light energy came. The precision ground glass may be added to the adhesive or the surface of the base material or may be coated on the surface of the base material.

The coextrusion, quenching, orienting, and heat setting of the polymer base sheet may be effected by any process which is known in the art for producing oriented sheet, such as by a flat sheet process or a bubble or tubular process. The flat sheet process involves extruding or coextruding the blend through a slit die and rapidly quenching the extruded or coextruded web upon a chilled casting drum so that the polymer component(s) of the sheet are quenched below their solidification temperature. The quenched base sheet is then biaxially oriented by stretching in mutually perpendicular directions at a temperature above the glass transition temperature of the polymer(s). The sheet may be stretched in one direction and then in a second direction or may be simultaneously stretched in both directions. After the sheet has been stretched, it is heat set by heating to a temperature sufficient to crystallize the polymers while restraining to some degree the sheet against retraction in both directions of stretching.

The base material of the invention in one preferred embodiment is provided with a metallic layer below the laminated developed imaging layers. The metallic layer provides a mirror like surface that is highly reflective and

has commercial value as metallic images are especially attractive to youth and commercial advertisements. The metallic layer is preferably applied to the base prior to lamination. A preferred example is a vacuum deposited layer of aluminum on a sheet of biaxially oriented polyolefin.

To adhere the transparent sheet with the developed image layers to the base sheet of the invention a bonding layer is required. The bonding layer must provide excellent adhesion between the imaging layers and the base sheet for the useful life of the image. The preferred method of adhering the imaging layers and the base sheet is by use of an adhesive. The adhesive preferably is coated or applied to the base sheet. The adhesive preferably is a pressure sensitive adhesive or heat activated adhesive. During the bonding process, the imaging layers is adhered to the base by use of a nip roller or a heated nip roll in the case of a heat activated adhesive. A preferred pressure sensitive adhesive is an acrylic based adhesive. Acrylic adhesives have been shown to provide an excellent bond between gelatin developed imaging layers and biaxially oriented polymer base sheets.

The preferred thickness of the adhesive layer is between 2 and 40 micrometers. Below 1 micrometer, uniformity of the adhesive is difficult to maintain leading to undesirable coating skips. Above 45 micrometers, little improvement is 25 adhesion and coating quality is observed and therefore thicker coatings are not cost justified. An important property of the adhesion layer between the developed silver halide imaging layers and the base material is the optical transmission of the adhesive layer. A laminated adhesive layer with an optical transmission greater than 90% is preferred as the adhesive should not interfere with the quality of the image.

The following is a preferred structure of an exposed, developed and laminated silver halide depth image. In the 35 following preferred depth imaging structure the silver halide imaging layers were curtain coated on to the gelatin sub coated transparent polyester sheet. The silver halide images were printed and developed using standard processing chemistry. The developed images were then adhered to a reflective white base using an acrylic pressure sensitive 40 adhesive:

---

|    |                                                           |
|----|-----------------------------------------------------------|
| 45 | Developed silver halide imaging layers                    |
|    | Gelatin sub coating                                       |
|    | Oriented polyester                                        |
|    | Gelatin sub coating                                       |
| 50 | Developed silver halide imaging layers                    |
|    | Acrylic adhesive with 0.20% optical brightener            |
|    | Polypropylene with blue tint, 24% rutile TiO <sub>2</sub> |
|    | Oriented, voided polypropylene                            |
|    | Polypropylene                                             |

---

Disclosed below is a suitable flesh tone optimized light sensitive silver halide emulsion capable of accurately reproducing flesh tones. Other suitable silver halide imaging layers also could be utilized in the invention photographic element. This preferred emulsion for the invention is directed to a silver halide depth image of excellent performance when exposed by either an electronic printing method 55 or a conventional optical printing method. An electronic printing method comprises subjecting a radiation sensitive silver halide emulsion layer of a recording element to actinic radiation of at least 10<sup>-4</sup> ergs/cm<sup>2</sup> for up to 100 $\mu$  seconds duration in a pixel-by-pixel mode wherein the silver halide emulsion layer is comprised of silver halide grains as described above. A conventional optical printing method 60 comprises subjecting a radiation sensitive silver halide emulsion layer to a radiation source having a wavelength of 365 nm for a duration of 100 seconds.

emulsion layer of a recording element to actinic radiation of at least  $10^{-4}$  ergs/cm<sup>2</sup> for  $10^{-3}$  to 300 seconds in an imagewise mode wherein the silver halide emulsion layer is comprised of silver halide grains as described above.

It has been found that the duplitized emulsion coverage for the three dimensional image or the application of silver halide imaging layers to both the top and bottom of the transparent sheet, should be in a range that is greater than 60% and less than 125% of the of typically emulsion coverage for reflective consumer paper that contain typical amounts of silver and coupler. It has been shown that the top side emulsion coverage or the exposed emulsion after printing, of 125% for the typical emulsion coverage resulted in significant and adverse attenuation of the imaging light which resulted in under exposure of the bottom side emulsion coating or the emulsion adhered to the reflective support. Conversely, imaging through the 60% bottom coverage resulted in significant and adverse attenuation of the imaging light which resulted in over exposure of the top side emulsion coating.

The depth imaging material of this invention wherein at least one dye forming coupler on the bottom side of the imaging support has less dye forming coupler than the imaging layer on the top side is preferred because it allows for an increase in image density without increasing developer time. The depth imaging material of this invention wherein the amount of dye forming coupler is substantially the same on the top and bottom sides is most preferred because it allows for optimization of image density while allowing for developer time less than 50 seconds. Further, coating substantially the same amount of light sensitive silver halide emulsion on both sides has the additional benefit of balancing the imaging element for image curl caused by the contraction and expansion of the hydroscopic gel typically found in photographic emulsions.

This invention in a preferred embodiment utilizes a radiation-sensitive emulsion comprised of silver halide grains (a) containing greater than 50 mole percent chloride, based on silver, (b) having greater than 50 percent of their surface area provided by {100} crystal faces, and (c) having a central portion accounting for from 95 to 99 percent of total silver and containing two dopants selected to satisfy each of the following class requirements: (i) a hexacoordination metal complex which satisfies the formula



wherein n is zero, -1, -2, -3 or -4; M is a filled frontier orbital polyvalent metal ion, other than iridium; and L<sub>6</sub> represents bridging ligands which can be independently selected, provided that least four of the ligands are anionic ligands, and at least one of the ligands is a cyano ligand or a ligand more electronegative than a cyano ligand; and (ii) an iridium coordination complex containing a thiazole or substituted thiazole ligand.

This invention is directed towards a photographic label comprising a flexible substrate and at least one light sensitive silver halide emulsion layer comprising silver halide grains as described above. The photographic label may be color or black and white where silver is retained in the developed imaging layer to form density.

It has been discovered quite surprisingly that the combination of dopants (i) and (ii) provides greater reduction in reciprocity law failure than can be achieved with either dopant alone. Further, unexpectedly, the combination of dopants (i) and (ii) achieve reductions in reciprocity law failure beyond the simple additive sum achieved when

employing either dopant class by itself. It has not been reported or suggested prior to this invention that the combination of dopants (i) and (ii) provides greater reduction in reciprocity law failure, particularly for high intensity and short duration exposures. The combination of dopants (i) and (ii) further unexpectedly achieves high intensity reciprocity with iridium at relatively low levels, and both high and low intensity reciprocity improvements even while using conventional gelatino-peptizer (e.g., other than low methionine gelatino-peptizer).

In a preferred practical application, the advantages of the invention can be transformed into increased throughput of digital substantially artifact-free color print images while exposing each pixel sequentially in synchronism with the digital data from an image processor.

In one embodiment, the present invention represents an improvement on the electronic printing method. Specifically, this invention in one embodiment is directed to an electronic printing method which comprises subjecting a radiation sensitive silver halide emulsion layer of a recording element to actinic radiation of at least  $10^{-4}$  ergs/cm<sup>2</sup> for up to  $100\mu$  seconds duration in a pixel-by-pixel mode. The present invention realizes an improvement in reciprocity failure by selection of the radiation sensitive silver halide emulsion layer. While certain embodiments of the invention are specifically directed towards electronic printing, use of the emulsions and elements of the invention is not limited to such specific embodiment, and it is specifically contemplated that the emulsions and elements of the invention are also well suited for conventional optical printing.

It has been unexpectedly discovered that significantly improved reciprocity performance can be obtained for silver halide grains (a) containing greater than 50 mole percent chloride, based on silver, and (b) having greater than 50 percent of their surface area provided by {100} crystal faces

by employing a hexacoordination complex dopant of class (i) in combination with an iridium complex dopant comprising a thiazole or substituted thiazole ligand. The reciprocity improvement is obtained for silver halide grains employing conventional gelatino-peptizer, unlike the contrast improvement described for the combination of dopants set forth in U.S. Pat. Nos. 5,783,373 and 5,783,378, which requires the use of low methionine gelatino-peptizers as discussed therein, and which states it is preferable to limit the concentration of any gelatino-peptizer with a methionine level of greater than 30 micromoles per gram to a concentration of less than 1 percent of the total peptizer employed. Accordingly, in specific embodiments of the invention, it is specifically contemplated to use significant levels (i.e., greater than 1 weight percent of total peptizer) of conventional gelatin (e.g., gelatin having at least 30 micromoles of methionine per gram) as a gelatino-peptizer for the silver halide grains of the emulsions of the invention. In preferred embodiments of the invention, gelatino-peptizer is employed which comprises at least 50 weight percent of gelatin containing at least 30 micromoles of methionine per gram, as it is frequently desirable to limit the level of oxidized low methionine gelatin which may be used for cost and certain performance reasons.

In a specific, preferred form of the invention it is contemplated to employ a class (i) hexacoordination complex dopant satisfying the formula:



where

n is zero, -1, -2, -3 or -4;  
M is a filled frontier orbital polyvalent metal ion, other than iridium, preferably  $Fe^{+2}$ ,  $Ru^{+32}$ ,  $Os^{+2}$ ,  $Co^{+3}$ ,  $Rh^{+3}$ ,  $Pd^{+4}$

or  $\text{Pt}^{+4}$ , more preferably an iron, ruthenium or osmium ion, and most preferably a ruthenium ion;

$L_6$  represents six bridging ligands which can be independently selected, provided that at least four of the ligands are anionic ligands and at least one (preferably at least 3 and optimally at least 4) of the ligands is a cyano ligand or a ligand more electronegative than a cyano ligand. Any remaining ligands can be selected from among various other bridging ligands, including aquo ligands, halide ligands (specifically, fluoride, chloride, bromide and iodide), cyanate ligands, thiocyanate ligands, selenocyanate ligands, tellurocyanate ligands, and azide ligands. Hexacoordinated transition metal complexes of class (i) which include six cyano ligands are specifically preferred.

Illustrations of specifically contemplated class (i) hexacoordination complexes for inclusion in the high chloride grains are provided by Olm et al U.S. Pat. No. 5,503,970 and Daubendiek et al U.S. Pat. Nos. 5,494,789 and 5,503,971, and Keevert et al U.S. Pat. No. 4,945,035, as well as Murakami et al Japanese Patent Application Hei-2[1990]-249588, and Research Disclosure Item 36736. Useful neutral and anionic organic ligands for class (ii) dopant hexacoordination complexes are disclosed by Olm et al U.S. Pat. No. 5,360,712 and Kuromoto et al U.S. Pat. No. 5,462,849.

Class (i) dopant is preferably introduced into the high chloride grains after at least 50 (most preferably 75 and optimally 80) percent of the silver has been precipitated, but before precipitation of the central portion of the grains has been completed. Preferably class (i) dopant is introduced before 98 (most preferably 95 and optimally 90) percent of the silver has been precipitated. Stated in terms of the fully precipitated grain structure, class (i) dopant is preferably present in an interior shell region that surrounds at least 50 (most preferably 75 and optimally 80) percent of the silver and, with the more centrally located silver, accounts the entire central portion (99 percent of the silver), most preferably accounts for 95 percent, and optimally accounts for 90 percent of the silver halide forming the high chloride grains. The class (i) dopant can be distributed throughout the interior shell region delimited above or can be added as one or more bands within the interior shell region.

Class (i) dopant can be employed in any conventional useful concentration. A preferred concentration range is from  $10^{-8}$  to  $10^{-3}$  mole per silver mole, most preferably from  $10^{-6}$  to  $5 \times 10^{-4}$  mole per silver mole.

The following are specific illustrations of class (i) dopants:

- (i-1)  $[\text{Fe}(\text{CN})_6]^{-4}$
- (i-2)  $[\text{Ru}(\text{CN})_6]^{-4}$
- (i-3)  $[\text{Os}(\text{CN})_6]^{-4}$
- (i-4)  $[\text{Rh}(\text{CN})_6]^{-3}$
- (i-5)  $[\text{Co}(\text{CN})_6]^{-3}$
- (i-6)  $[\text{Fe}(\text{pyrazine})(\text{CN})_5]^{-4}$
- (i-7)  $[\text{RuCl}(\text{CN})_5]^{-4}$
- (i-8)  $[\text{OsBr}(\text{CN})_5]^{-4}$
- (i-9)  $[\text{RhF}(\text{CN})_5]^{-3}$
- (i-10)  $[\text{In}(\text{NCS})_6]^{-3}$
- (i-11)  $[\text{FeCO}(\text{CN})_5]^{-3}$
- (i-12)  $[\text{RuF}_2(\text{CN})_4]^{-4}$
- (i-13)  $[\text{OsCl}_2(\text{CN})_4]^{-4}$
- (i-14)  $[\text{RhI}_2(\text{CN})_4]^{-3}$
- (i-15)  $[\text{Ga}(\text{NCS})_6]^{-3}$
- (i-16)  $[\text{Ru}(\text{CN})_5(\text{OCN})]^{-4}$

- (i-17)  $[\text{Ru}(\text{CN})_5(\text{N}_3)]^{-4}$
- (i-18)  $[\text{Os}(\text{CN})_5(\text{SCN})]^{-4}$
- (i-19)  $[\text{Rh}(\text{CN})_5(\text{SeCN})]^{-3}$
- (i-20)  $[\text{Os}(\text{CN})\text{Cl}_5]^{-4}$
- (i-21)  $[\text{Fe}(\text{CN})_3\text{Cl}_3]^{-3}$
- (i-22)  $[\text{Ru}(\text{CO})_2(\text{CN})_4]^{-1}$

When the class (i) dopants have a net negative charge, it is appreciated that they are associated with a counter ion when added to the reaction vessel during precipitation. The counter ion is of little importance since it is tonically dissociated from the dopant in solution and is not incorporated within the grain. Common counter ions known to be fully compatible with silver chloride precipitation, such as ammonium and alkali metal ions, are contemplated. It is noted that the same comments apply to class (ii) dopants, otherwise described below.

The class (ii) dopant is an iridium coordination complex containing at least one thiazole or substituted thiazole ligand. Careful scientific investigations have revealed Group VIII hexahalo coordination complexes to create deep electron traps, as illustrated R. S. Eachus, R. E. Graves and M. T. Olm *J. Chem. Phys.*, Vol. 69, pp. 4580-7 (1978) and *Physica Status Solidi A*, Vol. 57, 429-37 (1980) and R. S. Eachus and M. T. Olm *Annu. Rep. Prog. Chem. Sect. C. Phys. Chem.*, Vol. 83, 3, pp. 3-48 (1986). The class (ii) dopants employed in the practice of this invention are believed to create such deep electron traps. The thiazole ligands may be substituted with any photographically acceptable substituent which does not prevent incorporation of the dopant into the silver halide grain. Exemplary substituents include lower alkyl (e.g., alkyl groups containing 1-4 carbon atoms), and specifically methyl. A specific example of a substituted thiazole ligand which may be used in accordance with the invention is 5-methylthiazole. The class (ii) dopant preferably is an iridium coordination complex having ligands each of which are more electropositive than a cyano ligand. In a specifically preferred form the remaining non-thiazole or non-substituted-thiazole ligands of the coordination complexes forming class (ii) dopants are halide ligands.

It is specifically contemplated to select class (ii) dopants from among the coordination complexes containing organic ligands disclosed by Olm et al U.S. Pat. No. 5,360,712; Olm et al U.S. Pat. No. 5,457,021; and Kuromoto et al U.S. Pat. No. 5,462,849.

In a preferred form it is contemplated to employ as a class (ii) dopant a hexacoordination complex satisfying the formula:



wherein

$n'$  is zero, -1, -2, -3 or -4; and

$L_6$  represents six bridging ligands which can be independently selected, provided that at least four of the ligands are anionic ligands, each of the ligands is more electropositive than a cyano ligand, and at least one of the ligands comprises a thiazole or substituted thiazole ligand. In a specifically preferred form at least four of the ligands are halide ligands, such as chloride or bromide ligands.

Class (ii) dopant is preferably introduced into the high chloride grains after at least 50 (most preferably 85 and optimally 90) percent of the silver has been precipitated, but before precipitation of the central portion of the grains has been completed. Preferably class (ii) dopant is introduced

before 99 (most preferably 97 and optimally 95) percent of the silver has been precipitated. Stated in terms of the fully precipitated grain structure, class (ii) dopant is preferably present in an interior shell region that surrounds at least 50 (most preferably 85 and optimally 90) percent of the silver and, with the more centrally located silver, accounts for the entire central portion (99 percent of the silver), most preferably accounts for 97 percent, and optimally accounts for 95 percent of the silver halide forming the high chloride grains. The class (ii) dopant can be distributed throughout the interior shell region delimited above or can be added as one or more bands within the interior shell region.

Class (ii) dopant can be employed in any conventional useful concentration. A preferred concentration range is from  $10^{-9}$  to  $10^{-4}$  mole per silver mole. Iridium is most preferably employed in a concentration range of from  $10^{-8}$  to  $10^{-5}$  mole per silver mole.

Specific illustrations of class (ii) dopants are the following:

- (ii-1)  $[\text{IrCl}_5(\text{thiazole})]^{-2}$
- (ii-2)  $[\text{IrCl}_4(\text{thiazole})_2]^{-1}$
- (ii-3)  $[\text{IrBr}_5(\text{thiazole})]^{-2}$
- (ii-4)  $[\text{IrBr}_4(\text{thiazole})_2]^{-1}$
- (ii-5)  $[\text{IrCl}_5(5\text{-methylthiazole})]^{-2}$
- (ii-6)  $[\text{IrCl}_4(5\text{-methylthiazole})_2]^{-1}$
- (ii-7)  $[\text{IrBr}_5(5\text{-methylthiazole})]^{-2}$
- (ii-8)  $[\text{IrBr}_4(5\text{-methylthiazole})_2]^{-1}$

In one preferred aspect of the invention in a layer using a magenta dye forming coupler, a class (ii) dopant in combination with an  $\text{OsCl}_5(\text{NO})$  dopant has been found to produce a preferred result.

Emulsions demonstrating the advantages of the invention can be realized by modifying the precipitation of conventional high chloride silver halide grains having predominantly (>50%) {100} crystal faces by employing a combination of class (i) and (ii) dopants as described above.

The silver halide grains precipitated contain greater than 50 mole percent chloride, based on silver. Preferably the grains contain at least 70 mole percent chloride and, optimally at least 90 mole percent chloride, based on silver. Iodide can be present in the grains up to its solubility limit, which is in silver iodochloride grains, under typical conditions of precipitation, about 11 mole percent, based on silver. It is preferred for most photographic applications to limit iodide to less than 5 mole percent iodide, most preferably less than 2 mole percent iodide, based on silver.

Silver bromide and silver chloride are miscible in all proportions. Hence, any portion, up to 50 mole percent, of the total halide not accounted for chloride and iodide, can be bromide. For color reflection print (i.e., color paper) uses bromide is typically limited to less than 10 mole percent based on silver and iodide is limited to less than 1 mole percent based on silver.

In a widely used form high chloride grains are precipitated to form cubic grains—that is, grains having {100} major faces and edges of equal length. In practice ripening effects usually round the edges and corners of the grains to some extent. However, except under extreme ripening conditions substantially more than 50 percent of total grain surface area is accounted for by {100} crystal faces.

High chloride tetradechedahedral grains are a common variant of cubic grains. These grains contain 6 {100} crystal faces and 8 {111} crystal faces. Tetradechedahedral grains are within the contemplation of this invention to the extent that greater than 50 percent of total surface area is accounted for by {100} crystal faces.

Although it is common practice to avoid or minimize the incorporation of iodide into high chloride grains employed in color paper, it is has been recently observed that silver iodochloride grains with {100} crystal faces and, in some instances, one or more {111} faces offer exceptional levels of photographic speed. In these emulsions iodide is incorporated in overall concentrations of from 0.05 to 3.0 mole percent, based on silver, with the grains having a surface shell of greater than 50 Å that is substantially free of iodide and a interior shell having a maximum iodide concentration that surrounds a core accounting for at least 50 percent of total silver. Such grain structures are illustrated by Chen et al EPO 0 718 679.

In another improved form the high chloride grains can take the form of tabular grains having {100} major faces. Preferred high chloride {100} tabular grain emulsions are those in which the tabular grains account for at least 70 (most preferably at least 90) percent of total grain projected area. Preferred high chloride {100} tabular grain emulsions have average aspect ratios of at least (most preferably at least >8). Tabular grains typically have thicknesses of less than 0.3  $\mu\text{m}$ , preferably less than 0.2  $\mu\text{m}$ , and optimally less than 0.07  $\mu\text{m}$ . High chloride {100} tabular grain emulsions and their preparation are disclosed by Maskasky U.S. Pat. Nos. 5,264,337 and 5,292,632; House et al U.S. Pat. No. 5,320,938; Brust et al U.S. Pat. No. 5,314,798; and Chang et al U.S. Pat. No. 5,413,904.

Once high chloride grains having predominantly {100} crystal faces have been precipitated with a combination of class (i) and class (ii) dopants described above, chemical and spectral sensitization, followed by the addition of conventional addenda to adapt the emulsion for the imaging application of choice can take any convenient conventional form. These conventional features are illustrated by *Research Disclosure*, Item 38957, cited above, particularly:

- III. Emulsion washing;
- IV. Chemical sensitization;
- V. Spectral sensitization and desensitization;
- VII. Antifoggants and stabilizers;
- VIII. Absorbing and scattering materials;
- IX. Coating and physical property modifying addenda; and
- X. Dye image formers and modifiers.

Some additional silver halide, typically less than 1 percent, based on total silver, can be introduced to facilitate chemical sensitization. It is also recognized that silver halide can be epitaxially deposited at selected sites on a host grain to increase its sensitivity. For example, high chloride {100} tabular grains with corner epitaxy are illustrated by Maskasky U.S. Pat. No. 5,275,930. For the purpose of providing a clear demarcation, the term "silver halide grain" is herein employed to include the silver necessary to form the grain up to the point that the final {100} crystal faces of the grain are formed. Silver halide later deposited that does not overlie the {100} crystal faces previously formed accounting for at least 50 percent of the grain surface area is excluded in determining total silver forming the silver halide grains. Thus, the silver forming selected site epitaxy is not part of the silver halide grains while silver halide that deposits and provides the final {100} crystal faces of the grains is included in the total silver forming the grains, even when it differs significantly in composition from the previously precipitated silver halide.

Image dye-forming couplers may be included in the element such as couplers that form cyan dyes upon reaction with oxidized color developing agents which are described

in such representative patents and publications as: U.S. Pat. Nos. 2,367,531; 2,423,730; 2,474,293; 2,772,162; 2,895,826; 3,002,836; 3,034,892; 3,041,236; 4,883,746 and "Farbkuppler—Fine Literature Ubersicht," published in Agfa Mitteilungen, Band III, pp. 156-175 (1961). Preferably such couplers are phenols and naphthols that form cyan dyes on reaction with oxidized color developing agent. Also preferable are the cyan couplers described in, for instance, European Patent Application Nos. 491,197; 544,322; 556,700; 556,777; 565,096; 570,006; and 574,948.

Typical cyan couplers are represented by the following formulas:



wherein R<sub>1</sub>, R<sub>5</sub> and R<sub>8</sub> each represent a hydrogen or a substituent; R<sub>2</sub> represents a substituent; R<sub>3</sub>, R<sub>4</sub> and R<sub>7</sub> each represent an electron attractive group having a Hammett's substituent constant  $\sigma_{para}$  of 0.2 or more and the sum of the  $\sigma_{para}$  values of R<sub>3</sub> and R<sub>4</sub> is 0.65 or more; R<sub>6</sub> represents an electron attractive group having a Hammett's substituent constant  $\sigma_{para}$  of 0.35 or more; X represents a hydrogen or a coupling-off group; Z<sub>1</sub> represents nonmetallic atoms necessary for forming a nitrogen-containing, six-membered, heterocyclic ring which has at least one dissociative group; Z<sub>2</sub> represents  $-\text{C}(\text{R}_7)=$  and  $-\text{N}=\text{}$ ; and Z<sub>3</sub> and Z<sub>4</sub> each represent  $-\text{C}(\text{R}_8)=$  and  $-\text{N}=\text{}$ .

For purposes of this invention, an "NB coupler" is a dye-forming coupler which is capable of coupling with the developer 4-amino-3-methylthyl-N-ethyl-N-(2-methanesulfonamidoethyl) aniline sesquisulfate hydrate to form a dye for which the left bandwidth (LBW) of its absorption spectra upon "spin coating" of a 3% w/v solution of the dye in di-n-butyl sebacate solvent is at least 5 nm. less than the LBW for a 3% w/v solution of the same dye in acetonitrile. The LBW of the spectral curve for a dye is the distance between the left side of the spectral curve and the wavelength of maximum absorption measured at a density of half the maximum.

The "spin coating" sample is prepared by first preparing a solution of the dye in di-n-butyl sebacate solvent (3% w/v). If the dye is insoluble, dissolution is achieved by the

addition of some methylene chloride. The solution is filtered and 0.1-0.2ml is applied to a clear polyethylene terephthalate support (approximately 4 cm×4 cm) and spun at 4,000 RPM using the Spin Coating equipment, Model No. EC101, available from Headway Research Inc., Garland, Tex. The transmission spectra of the so prepared dye samples are then recorded.

Preferred "NB couplers" form a dye which, in n-butyl sebacate, has a LBW of the absorption spectra upon "spin coating" which is at least 15 nm, preferably at least 25 nm, less than that of the same dye in a 3% solution (w/v) in acetonitrile.

In a preferred embodiment the cyan dye-forming "NB coupler" useful in the invention has the formula (IA)



wherein

R' and R'' are substituents selected such that the coupler is a "NB coupler", as herein defined; and

Z is a hydrogen atom or a group which can be split off by the reaction of the coupler with an oxidized color developing agent.

The coupler of formula (IA) is a 2,5-diamido phenolic cyan coupler wherein the substituents R' and R'' are preferably independently selected from unsubstituted or substituted alkyl, aryl, amino, alkoxy and heterocycl groups.

In a further preferred embodiment, the "NB coupler" has the formula (I):



wherein

R'' and R''' are independently selected from unsubstituted or substituted alkyl, aryl, amino, alkoxy and heterocyclic groups and Z is as hereinbefore defined;

R<sub>1</sub> and R<sub>2</sub> are independently hydrogen or an unsubstituted or substituted alkyl group; and

Typically, R'' is an alkyl, amino or aryl group, suitably a phenyl group. R''' is desirably an alkyl or aryl group or a 5-10 membered heterocyclic ring which contains one or more heteroatoms selected from nitrogen, oxygen and sulfur, which ring group is unsubstituted or substituted.

In the preferred embodiment the coupler of formula (I) is a 2,5-diamido phenol in which the 5-amido moiety is an amide of a carboxylic acid which is substituted in the alpha position by a particular sulfone ( $-\text{SO}_2-$ ) group, such as, for example, described in U.S. Pat. No. 5,686,235. The sulfone moiety is an unsubstituted or substituted alkylsulfone or a

heterocycll sulfone or it is an arylsulfone, which is preferably substituted, in particular in the meta and/or para position.

Couplers having these structures of formulae (I) or (IA) comprise cyan dye-forming "NB couplers" which form image dyes having very sharp-cutting dye hues on the short wavelength side of the absorption curves with absorption maxima ( $\lambda_{max}$ ) which are shifted hypsochromically and are generally in the range of 620-645 nm, which is ideally suited for producing excellent color reproduction and high color saturation in color photographic packaging labels.

Referring to formula (I), R<sub>1</sub> and R<sub>2</sub> are independently hydrogen or an unsubstituted or substituted alkyl group, preferably having from 1 to 24 carbon atoms and in particular 1 to 10 carbon atoms, suitably a methyl, ethyl, n-propyl, isopropyl, butyl or decyl group or an alkyl group substituted with one or more fluoro, chloro or bromo atoms, such as a trifluoromethyl group. Suitably, at least one of R<sub>1</sub> and R<sub>2</sub> is a hydrogen atom and if only one of R<sub>1</sub> and R<sub>2</sub> is a hydrogen atom then the other is preferably an alkyl group having 1 to 4 carbon atoms, more preferably one to three carbon atoms and desirably two carbon atoms.

As used herein and throughout the specification unless where specifically stated otherwise, the term "alkyl" refers to an unsaturated or saturated straight or branched chain alkyl group, including alkenyl, and includes aralkyl and cyclic alkyl groups, including cycloalkenyl, having 3-8 carbon atoms and the term 'aryl' includes specifically fused aryl.

In formula (I), R" is suitably an unsubstituted or substituted amino, alkyl or aryl group or a 5-10 membered heterocyclic ring which contains one or more heteroatoms selected from nitrogen, oxygen and sulfur, which ring is unsubstituted or substituted, but is more suitably an unsubstituted or substituted phenyl group.

Examples of suitable substituent groups for this aryl or heterocyclic ring include cyano, chloro, fluoro, bromo, iodo, alkyl- or aryl-carbonyl, alkyl- or aryl-oxycarbonyl, carbonamido, alkyl- or aryl-carbonamido, alkyl- or aryl-sulfonyl, alkyl- or aryl-sulfonyloxy, alkyl- or aryl-oxysulfonyl, alkyl- or aryl-sulfoxide, alkyl- or aryl-sulfamoyl, alkyl- or aryl-sulfonamido, aryl, alkyl, alkoxy, aryloxy, nitro, alkyl- or aryl-ureido and alkyl- or aryl-carbamoyl groups, any of which may be further substituted. Preferred groups are halogen, cyano, alkoxy carbonyl, alkylsulfamoyl, alkyl-sulfonamido, alkylsulfonyl, carbamoyl, alkylcarbamoyl or alkylcarbonamido. Suitably, R" is a 4-chlorophenyl, 3,4-di-chlorophenyl, 3,4-difluorophenyl, 4-cyanophenyl, 3-chloro-4-cyanophenyl, pentafluorophenyl, or a 3- or 4-sulfonamidophenyl group.

In formula (I) when R" is alkyl, it may be unsubstituted or substituted with a substituent such as halogen or alkoxy. When R" is aryl or a heterocycle, it may be substituted. Desirably it is not substituted in the position alpha to the sulfonyl group.

In formula (I) when R" is a phenyl group, it may be substituted in the meta and/or para positions with one to three substituents independently selected from the group consisting of halogen, and unsubstituted or substituted alkyl, alkoxy, aryloxy, acyloxy, acylamino, alkyl- or aryl-sulfonyloxy, alkyl- or aryl-sulfamoyl, alkyl- or aryl-sulfamoylamino, alkyl- or aryl-sulfonamido, alkyl- or aryl-ureido, alkyl- or aryl-oxycarbonyl, alkyl- or aryl-oxycarbonylamino and alkyl- or aryl-carbamoyl groups.

In particular each substituent may be an alkyl group such as methyl, t-butyl, heptyl, dodecyl, pentadecyl, octadecyl or 1,1,2,2-tetramethylpropyl; an alkoxy group such as

methoxy, t-butoxy, octyloxy, dodecyloxy, tetradecyloxy, hexadecyloxy or octadecyloxy; an aryloxy group such as phenoxy, 4-t-butylphenoxy or 4-dodecyl-phenoxy; an alkyl- or aryl-acyloxy group such as acetoxy or dodecanoyloxy; an alkyl- or aryl-acylamino group such as acetamido, hexadecamido or benzamido; an alkyl- or aryl-sulfonyloxy group such as methyl-sulfonyloxy, dodecylsulfonyloxy or 4-methylphenyl-sulfonyloxy; an alkyl- or aryl-sulfamoyl group such as N-butylsulfamoyl or N-4-t-butylphenylsulfamoyl; an alkyl- or aryl-sulfamoylamino group such as N-butylsulfamoylamino or N-4-t-butylphenylsulfamoyl-amino; an alkyl- or aryl-sulfonamido group such as methane-sulfonamido, hexadecanesulfonamido or 4-chlorophenyl-sulfonamido; an alkyl- or arylureido group such as methylureido or phenylureido; an alkoxy- or aryloxy-carbonyl such as methoxycarbonyl or phenoxy carbonyl; an alkoxy- or aryloxy-carbonylamino group such as methoxy-carbonylamino or phenoxy-carbonylamino; an alkyl- or aryl-carbamoyl group such as N-butylcarbamoyl or N-methyl-N-dodecylcarbamoyl; or a perfluoroalkyl group such as trifluoromethyl or heptafluoropropyl.

Suitably the above substituent groups have 1 to 30 carbon atoms, more preferably 8 to 20 aliphatic carbon atoms. A desirable substituent is an alkyl group of 12 to 18 aliphatic carbon atoms such as dodecyl, pentadecyl or octadecyl or an alkoxy group with 8 to 18 aliphatic carbon atoms such as dodecyloxy and hexadecyloxy or a halogen such as a meta or para chloro group, carboxy or sulfonamido. Any such groups may contain interrupting heteroatoms such as oxygen to form e.g. polyalkylene oxides.

In formula (I) or (IA), Z is a hydrogen atom or a group which can be split off by the reaction of the coupler with an oxidized color developing agent, known in the photographic art as a 'coupling-off group' and may preferably be hydrogen, chloro, fluoro, substituted aryloxy or mercaptotetrazole, more preferably hydrogen or chlorine.

The presence or absence of such groups determines the chemical equivalency of the coupler, i.e., whether it is a 2-equivalent or 4-equivalent coupler, and its particular identity can modify the reactivity of the coupler. Such groups can advantageously affect the layer in which the coupler is coated, or other layers in the photographic recording material, by performing, after release from the coupler, functions such as dye formation, dye hue adjustment, development acceleration or inhibition, bleach acceleration or inhibition, electron transfer facilitation, color correction, and the like.

Representative classes of such coupling-off groups include, for example, halogen, alkoxy, aryloxy, heterocyclloxy, sulfonyloxy, acyloxy, acyl, heterocyclsulfonamido, heterocyclthio, benzothiazolyl, phosphonyloxy, alkylthio, arylthio, and arylazo. These coupling-off groups are described in the art, for example, in U.S. Pat. Nos. 2,455,169, 3,227,551, 3,432,521, 3,467,563, 3,617,291, 3,880,661, 4,052,212, and 4,134,766; and in U.K. Patent Nos. and published applications 1,466,728, 1,531,927, 1,533,039, 2,066,755A, and 2,017,704A, the disclosures of which are incorporated herein by reference. Halogen, alkoxy and aryloxy groups are most suitable.

Examples of specific coupling-off groups are —Cl, —F, —Br, —SCN, —OCH<sub>3</sub>, —OC<sub>6</sub>H<sub>5</sub>, —OCH<sub>2</sub>C(=O)NHCH<sub>2</sub>CH<sub>2</sub>OCH<sub>3</sub>, —OCH<sub>2</sub>C(=O)NHCH<sub>2</sub>CH<sub>2</sub>OCH<sub>3</sub>, —P(=O)(OC<sub>2</sub>H<sub>5</sub>)<sub>2</sub>, —SCH<sub>2</sub>CH<sub>2</sub>COOH,



and



Typically, the coupling-off group is a chlorine atom, hydrogen atom or p-methoxyphenoxy group.

It is essential that the substituent groups be selected so as to adequately ballast the coupler and the resulting dye in the organic solvent in which the coupler is dispersed. The ballasting may be accomplished by providing hydrophobic substituent groups in one or more of the substituent groups. Generally a ballast group is an organic radical of such size and configuration as to confer on the coupler molecule sufficient bulk and aqueous insolubility as to render the coupler substantially nondiffusible from the layer in which it is coated in a photographic element. Thus the combination of substituent are suitably chosen to meet these criteria. To be effective, the ballast will usually contain at least 8 carbon atoms and typically contains 10 to 30 carbon atoms. Suitable ballasting may also be accomplished by providing a plurality of groups which in combination meet these criteria. In the preferred embodiments of the invention  $R_1$  in formula (I) is

a small alkyl group or hydrogen. Therefore, in these embodiments the ballast would be primarily located as part of the other groups. Furthermore, even if the coupling-off group  $Z$  contains a ballast it is often necessary to ballast the other substituents as well, since  $Z$  is eliminated from the molecule upon coupling; thus, the ballast is most advantageously provided as part of groups other than  $Z$ .

The following examples further illustrate preferred coupler of the invention. It is not to be construed that the present invention is limited to these examples.



**23**

-continued

**24**

-continued



**25**

-continued



IC-15



IC-16



IC-17



IC-18

**26**

-continued

IC-19



IC-20



IC-21



IC-22

**27**

-continued



IC-23

5



IC-24

10



IC-25

15



20

IC-26

25

30

35

40

45

50

55

60

65

**28**

-continued

IC-27



IC-29



IC-30



**29**

-continued



IC-31

5



IC-32 20

25



IC-33 35

40



IC-34

55

**30**

-continued



IC-35



IC-36



IC-37



IC-38

31

-continued



IC-39 and IC-40 are variations of structure 31.

32

-continued

MAGENTA-2



wherein  $R_a$  and  $R_b$  independently represent H or a substituent;  $R_c$  is a substituent (preferably an aryl group);  $R_d$  is a substituent (preferably an anilino, carbonamido, ureido, carbamoyl, alkoxy, aryloxycarbonyl, alkoxy carbonyl, or N-heterocyclic group); X is hydrogen or a coupling-off group; and  $Z_a$ ,  $Z_b$ , and  $Z_c$  are independently a substituted methine group,  $=N-$ ,  $=C-$ , or  $—NH—$ , provided that one of either the  $Z_a-Z_b$  bond or the  $Z_b-Z_c$  bond is a double bond and the other is a single bond, and when the  $Z_b-Z_c$  bond is a carbon-carbon double bond, it may form part of an aromatic ring, and at least one of  $Z_a$ ,  $Z_b$ , and  $Z_c$  represents a methine group connected to the group  $R_b$ .

Specific examples of such couplers are:



Preferred couplers are IC-3, IC-7, IC-35, and IC-36 because of their suitably narrow left bandwidths.

Couplers that form magenta dyes upon reaction with oxidized color developing agent are described in such representative patents and publications as: U.S. Pat. Nos. 2,311,082; 2,343,703; 2,369,489; 2,600,788; 2,908,573; 3,062,653; 3,152,896; 3,519,429; 3,758,309; and “Farbkuppler-eine Literature Ubersicht,” published in Agfa Mitteilungen, Band III, pp. 126–156 (1961). Preferably such couplers are pyrazolones, pyrazolotriazoles, or pyrazolobenzimidazoles; that form magenta dyes upon reaction with oxidized color developing agents. Especially preferred couplers are 1H-pyrazolo[5,1-c]-1,2,4-triazole and 1H-pyrazolo[1,5-b]-1,2,4-triazole. Examples of 1H-pyrazolo[5,1-c]-1,2,4-triazole couplers are described in U.K. Patent Nos. 1,247,493; 1,252,418; 1,398,979; U.S. Pat. Nos. 4,443,536; 4,514,490; 4,540,654; 4,590,153; 4,665,015; 4,822,730; 4,945,034; 5,017,465; and 5,023,170. Examples of 1H-pyrazolo[1,5]-bi-1,2,4-triazoles can be found in European Patent Applications 176,804; 177,765; U.S. Pat. Nos. 4,659,652; 5,066,575; and 5,250,400.

Typical pyrazoloazole and pyrazolone couplers are represented by the following formulas:



MAGENTA-1

60

65

**33**

-continued

**34**

-continued

YELLOW-2



YELLOW-3

YELLOW-4

Couplers that form yellow dyes upon reaction with oxidized color developing agent are described in such representative patents and publications as: U.S. Pat. Nos. 2,298,443; 2,407,210; 2,875,057; 3,048,194; 3,265,506; 3,447,928; 3,960,570; 4,022,620; 4,443,536; 4,910,126; and 5,340,703 and "Farbkuppler-eine Literature Ubersicht," published in *Agfa Mitteilungen*, Band 111, pp. 112-126 (1961). Such couplers are typically open chain ketomethylene compounds. Also preferred are yellow couplers such as described in, for example, European Patent Application Nos. 482,552; 510,535; 524,540; 543,367; and U.S. Pat. No. 5,238,803. For improved color reproduction, couplers which give yellow dyes that cut off sharply on the long wavelength side are particularly preferred (for example, see U.S. Pat. No. 5,360,713).

Typical preferred yellow couplers are represented by the following formulas:

YELLOW-1



wherein R<sub>1</sub>, R<sub>2</sub>, Q<sub>1</sub> and Q<sub>2</sub> each represents a substituent; X is hydrogen or a coupling-off group; Y represents an aryl group or a heterocyclic group; Q<sub>3</sub> represents an organic residue required to form a nitrogen-containing heterocyclic group together with the >N—; and Q<sub>4</sub> represents nonmetallic atoms necessary to from a 3- to 5-membered hydrocarbon ring or a 3- to 5-membered heterocyclic ring which contains at least one hetero atom selected from N, O, S, and P in the ring. Particularly preferred is when Q<sub>1</sub> and Q<sub>2</sub> each represent an alkyl group, an aryl group, or a heterocyclic group, and R<sub>2</sub> represents an aryl or tertiary alkyl group.

Preferred yellow couplers can be of the following general structures

Y-1



-continued



Y-2



Y-3



Y-4



Y-5



-continued



Y-6

Unless otherwise specifically stated, substituent groups which may be substituted on molecules herein include any groups, whether substituted or unsubstituted, which do not destroy properties necessary for photographic utility. When the term "group" is applied to the identification of a substituent containing a substitutable hydrogen, it is intended to encompass not only the substituent's unsubstituted form, but also its form further substituted with any group or groups as herein mentioned. Suitably, the group may be halogen or may be bonded to the remainder of the molecule by an atom of carbon, silicon, oxygen, nitrogen, phosphorous, or sulfur. The substituent may be, for example, halogen, such as chlorine, bromine or fluorine; nitro; hydroxyl; cyano; carboxyl; or groups which may be further substituted, such as alkyl, including straight or branched chain alkyl, such as methyl, trifluoromethyl, ethyl, t-butyl, 3-(2,4-di-tert-pentylphenoxy)propyl, and tetradecyl; alkenyl, such as ethylene, 2-butene; alkoxy, such as methoxy, ethoxy, propoxy, butoxy, 2-methoxyethoxy, sec-butoxy, hexyloxy, 2-ethylhexyloxy, tetradecyloxy, 2-(2,4-di-tert-pentylphenoxy)ethoxy, and 2-dodecyloxyethoxy; aryl such as phenyl, 4-t-butylphenyl, 2,4,6-trimethylphenyl, naphthyl; aryloxy, such as phenoxy, 2-methylphenoxy, alpha- or beta-naphthoxy, and 4-tolyloxy; carbonamido, such as acetamido, benzamido, butyramido, tetradecanamido, alpha-(2,4-di-tert-pentyl-phenoxy)acetamido, alpha-(2,4-di-tert-pentylphenoxy)butyramido, alpha-(3-pentadecylphenoxy)-hexanamido, alpha-(4-hydroxy-3-tert-butylphenoxy)-tetradecanamido, 2-oxo-pyrrolidin-1-yl, 2-oxo-5-tetradecylpyrrolin-1-yl, N-methyltetradecanamido, N-succinimido, N-phthalimido, 2,5-dioxo-1-oxazolidinyl, 3-dodecyl-2,5-dioxo-1-imidazolyl, and N-acetyl-N-dodecylamino, 50 ethoxycarbonylamino, phenoxy carbonylamino, benzyloxycarbonylamino, hexadecyloxycarbonylamino, 2,4-di-tert-butylphenoxy carbonylamino, phenylcarbonylamino, 2,5-(di-tert-pentylphenyl) carbonylamino, p-dodecyl-phenylcarbonylamino, p-tolylcarbonylamino, N-methylureido, N,N-dimethylureido, N-methyl-N-dodecylureido, N,N-diethyl-N'-ethylureido, N-phenylureido, N,N-diphenylureido, N-phenyl-N-p-tolylureido, N-(m-hexadecylphenyl)ureido, N,N-(2,5-di-tert-pentylphenyl)-N'-ethylureido, and t-butylcarbonamido; sulfonamido, such as methylsulfonamido, benzenesulfonamido, p-tolylsulfonamido, p-dodecylbenzenesulfonamido, N-methyltetradecylsulfonamido, N,N-dipropylsulfamoylamino, and hexadecylsulfonamido; sulfamoyl, such as N-methylsulfamoyl, N-ethylsulfamoyl, N,N-dipropylsulfamoyl, N-hexadecylsulfamoyl, N,N-dimethylsulfamoyl; N-[3-(dodecyloxy)propyl]sulfamoyl, N-[4-(2,4-di-tert-pentylphenoxy)butyl]sulfamoyl, N-methyl-N-tetradecylsulfamoyl, and N-dodecylsulfamoyl; carbamoyl, such as N-methylcarbamoyl, N,N-dibutylcarbamoyl, N-octadecylcarbamoyl, N-[4-(2,4-di-tert-pentylphenoxy)butyl]carbamoyl, N-methyl-N-tetradecylcarbamoyl, and N,N-diethylcarbamoyl; acyl, such as acetyl, (2,4-di-tert-amylphenoxy)acetyl, phenoxy carbonyl, p-dodecyloxyphenoxy carbonyl, methoxycarbonyl, butoxycarbonyl, tetradecyloxy carbonyl, ethoxycarbonyl, benzyloxycarbonyl, 3-pentadecyloxy carbonyl, and dodecylloxycarbonyl; sulfonyl, such as methoxysulfonyl, octyloxysulfonyl, tetradecyloxysulfonyl, 2-ethylhexyloxysulfonyl, phenoxy sulfonyl, 2,4-di-tert-pentylphenoxy sulfonyl, methylsulfonyl, octylsulfonyl, 2-ethylhexylsulfonyl, dodecylsulfonyl, hexadecylsulfonyl, phenylsulfonyl, 4-nonylphenylsulfonyl, and p-tolylsulfonyl; sulfonyloxy, such as dodecylsulfonyloxy, and hexadecylsulfonyloxy; sulfinyl, such as methylsulfinyl, octylsulfinyl, 2-ethylhexylsulfinyl, dodecylsulfinyl, hexadecylsulfinyl, phenylsulfinyl, 4-nonylphenylsulfinyl, and p-tolylsulfinyl; thio, such as ethylthio, octylthio, benzylthio, tetradecylthio, 2-(2,4-di-tert-pentylphenoxy)ethylthio, phenylthio, 2-butoxy-5-tert-octylphenylthio, and p-tolylthio; acyloxy, such as acetoxy, benzyloxy, octadecanoxy, p-dodecylamidobenzoxyloxy, N-phenylcarbamoyloxy, N-ethylcarbamoyloxy, and cyclohexylcarbonyloxy; amino, such as phenylanilino, 2-chloroanilino, diethylamino, dodecylamino; imino, such as 1-(N-phenylimido)ethyl, N-succinimido or 3-benzylidantoinyl; phosphate, such as dimethylphosphate and ethylbutylphosphate; phosphite, such as diethyl and dihexylphosphite; a heterocyclic group, a heterocyclic oxy group or a heterocyclic thio group, each of which may be substituted and which contain a 3- to 7-membered heterocyclic ring composed of carbon atoms and at least one hetero atom selected from the group consisting of oxygen, nitrogen and sulfur, such as 2-furyl, 2-thienyl, 2-benzimidazolyl, or 2-benzothiazolyl; quaternary ammonium, such as triethylammonium; and silyloxy, such as trimethylsilyloxy.

If desired, the substituents may themselves be further substituted one or more times with the described substituent groups. The particular substituents used may be selected by those skilled in the art to attain the desired photographic properties for a specific application and can include, for example, hydrophobic groups, solubilizing groups, blocking groups, releasing or releasable groups, etc. Generally, the above groups and substituents thereof may include those

39

having up to 48 carbon atoms, typically 1 to 36 carbon atoms and usually less than 24 carbon atoms, but greater numbers are possible depending on the particular substituents selected.

Representative substituents on ballast groups include alkyl, aryl, alkoxy, aryloxy, alkylthio, hydroxy, halogen, alkoxy carbonyl, aryloxy carbonyl, carboxy, acyl, acyloxy, amino, anilino, carbonamido, carbamoyl, alkylsulfonyl, arylsulfonyl, sulfonamido, and sulfamoyl groups wherein the substituents typically contain 1 to 42 carbon atoms. Such substituents can also be further substituted.

40

Silver halide imaging layers substantially free of stabilizers are preferred. Silver halide stabilizers are typically utilized to protect from the growth of fog in storage and to reduce image fading. Stabilizers are however expensive and not generally required for silver halide images attached to packages of the invention since the shelf life of a package tends to be less than one calendar year. Silver halide imaging layers substantially free of stabilizers would be low in cost and have acceptable image quality for images attached to packages.

Stabilizers and scavengers that can be used in these photographic elements, but are not limited to, the following.



-continued

ST-11

ST-12



ST-13



ST-8



ST-14



ST-15

ST-16



ST-17



ST-18

ST-19



ST-20



43



0 NHBu-t 0  
n: m 1: 1 mw = 75–100,000

-continued

ST-21



ST-22

ST-23



ST-15



ST-16



ST-17



ST-18



ST-19



ST-20



n = 75 - 8,000



-continued

ST-21



ST-22



ST-23



ST-24



Examples of solvents which may be used in the invention include the following:

---

|                                                 |      |
|-------------------------------------------------|------|
| Tritolyl phosphate                              | S-1  |
| Dibutyl phthalate                               | S-2  |
| Diundecyl phthalate                             | S-3  |
| N,N-Diethyldodecanamide                         | S-4  |
| N,N-Dibutyldodecanamide                         | S-5  |
| Tris(2-ethylhexyl)phosphate                     | S-6  |
| Acetyl tributyl citrate                         | S-7  |
| 2,4-Di-tert-pentylphenol                        | S-8  |
| 2-(2-Butoxyethoxy)ethyl acetate                 | S-9  |
| 1,4-Cyclohexyldimethylene bis(2-ethylhexanoate) | S-10 |

---

The dispersions used in photographic elements may also include ultraviolet (UV) stabilizers and so called liquid UV stabilizers such as described in U.S. Pat. Nos. 4,992,358; 4,975,360; and 4,587,346. Examples of UV stabilizers are shown below.





-continued



Further, it is contemplated to stabilize photographic dispersions prone to particle growth through the use of hydrophobic, photographically inert compounds such as disclosed by Zengerle et al in U.S. Ser. No. 07/978,104.

In a preferred embodiment the invention employs recording elements which are constructed to contain at least three silver halide emulsion layer units. A suitable full color, multilayer format for a recording element used in the invention is represented by Structure I.



### STRUCTURE I

wherein the red-sensitized, cyan dye image-forming silver halide emulsion unit is situated nearest the support; next in order is the green-sensitized, magenta dye image-forming unit, followed by the uppermost blue-sensitized, yellow dye image-forming unit. The image-forming units are separated from each other by hydrophilic colloid interlayers containing an oxidized developing agent scavenger to prevent color contamination. Silver halide emulsions satisfying the grain and gelatino-peptizer requirements described above can be present in any one or combination of the emulsion layer units. Additional useful multicolor, multilayer formats for an element of the invention include structures as described in U.S. Pat. No. 5,783,373. Each of such structures in accordance with the invention preferably would contain at least three silver halide emulsions comprised of high chloride grains having at least 50 percent of their surface area bounded by {100} crystal faces and containing dopants from classes (i) and (ii), as described above. Preferably each of the emulsion layer units contains emulsion satisfying these criteria.

Conventional features that can be incorporated into multilayer (and particularly multicolor) recording elements contemplated for use in the method of the invention are illustrated by *Research Disclosure*, Item 38957, cited above:

XI. Layers and layer arrangements

XII. Features applicable only to color negative

XIII. Features applicable only to color positive

B. Color reversal

C. Color positives derived from color negatives

XIV. Scan facilitating features.

The recording elements comprising the radiation sensitive high chloride emulsion layers according to this invention can be conventionally optically printed, or in accordance with a particular embodiment of the invention can be image-wise exposed in a pixel-by-pixel mode using suitable high energy radiation sources typically employed in electronic printing methods. Suitable actinic forms of energy encompass the ultraviolet, visible and infrared regions of the electromagnetic spectrum as well as electron-beam radiation and is conveniently supplied by beams from one or more light emitting diodes or lasers, including gaseous or solid state lasers. Exposures can be monochromatic, orthochromatic or panchromatic. For example, when the recording element is a multilayer multicolor element, exposure can be provided by laser or light emitting diode beams of appropriate spectral radiation, for example, infrared, red, green or blue wavelengths, to which such element is sensitive. Multicolor elements can be employed which produce cyan, magenta and yellow dyes as a function of exposure in separate portions of the electromagnetic spectrum, including at least two portions of the infrared region, as disclosed in the previously mentioned U.S. Pat. No. 4,619,892. Suitable exposures include those up to 2000 nm, preferably up to 1500 nm. Suitable light emitting diodes and commercially available laser sources are known and commercially available. Image-wise exposures at ambient, elevated or reduced temperatures and/or pressures can be employed within the useful response range of the recording element determined by conventional sensitometric techniques, as illustrated by T. H. James, *The Theory of the Photographic Process*, 4th Ed., Macmillan, 1977, Chapters 4, 6, 17, 18 and 23.

It has been observed that anionic  $[MX_xY_yL_z]$  hexacoordination complexes, where M is a group 8 or 9 metal (preferably iron, ruthenium or iridium), X is halide or pseudohalide (preferably Cl, Br or CN) x is 3 to 5, Y is  $H_2O$ , y is 0 or 1, L is a C—C, H—C or C—N—H organic ligand, and Z is 1 or 2, are surprisingly effective in reducing high intensity reciprocity failure (HIRF), low intensity reciprocity failure (LIRF) and thermal sensitivity variance and in improving latent image keeping (LIK). As herein employed HIRF is a measure of the variance of photographic properties for equal exposures, but with exposure times ranging from  $10^{-1}$  to  $10^{-6}$  second. LIRF is a measure of the variance of photographic properties for equal exposures, but with exposure times ranging from  $10^{-1}$  to 100 seconds. Although these advantages can be generally compatible with face centered cubic lattice grain structures, the most striking improvements have been observed in high (>50 mole %, preferably  $\geq 90$  mole %) chloride emulsions. Preferred C—C, H—C or C—N—H organic ligands are aromatic heterocycles of the type described in U.S. Pat. No. 5,462,849. The most effective C—C, H—C or C—N—H organic ligands are azoles and azines, either unsubstituted or containing alkyl, alkoxy or halide substituents, where the alkyl moieties contain from 1 to 8 carbon atoms. Particularly preferred azoles and azines include thiazoles, thiazolines, and pyrazines.

The quantity or level of high energy actinic radiation provided to the recording medium by the exposure source is generally at least  $10^{-4}$  ergs/cm<sup>2</sup>, typically in the range about  $10^{-4}$  ergs/cm<sup>2</sup> to  $10^{-3}$  ergs/cm<sup>2</sup> and often from  $10^{-3}$  ergs/cm<sup>2</sup> to  $10^2$  ergs/cm<sup>2</sup>. Exposure of the recording element in a pixel-by-pixel mode as known in the prior art persists for only a very short duration or time. Typical maximum

exposure times are up to  $100\mu$  seconds, often up to  $10\mu$  seconds, and frequently up to only  $0.5\mu$  seconds. Single or multiple exposures of each pixel are contemplated. The pixel density is subject to wide variation, as is obvious to those skilled in the art. The higher the pixel density, the sharper the images can be, but at the expense of equipment complexity. In general, pixel densities used in conventional electronic printing methods of the type described herein do not exceed  $10^7$  pixels/cm<sup>2</sup> and are typically in the range of about  $10^4$  to  $10^6$  pixels/cm<sup>2</sup>. An assessment of the technology of high-quality, continuous-tone, color electronic printing using silver halide photographic paper which discusses various features and components of the system, including exposure source, exposure time, exposure level and pixel density and other recording element characteristics is provided in Firth et al., *A Continuous-Tone Laser Color Printer*, Journal of Imaging Technology, Vol. 14, No. 3, June 1988, which is hereby incorporated herein by reference. As previously indicated herein, a description of some of the details of conventional electronic printing methods comprising scanning a recording element with high energy beams such as light emitting diodes or laser beams, are set forth in Hioki U.S. Pat. No. 5,126,235, European Patent Applications 479 1567 A1 and 502 508 A1.

Once imagewise exposed, the recording elements can be processed in any convenient conventional manner to obtain a viewable image. Such processing is illustrated by *Research Disclosure*, Item 38957, cited above:

XVIII. Chemical development systems

XIX. Development

XX. Desilvering, washing, rinsing and stabilizing

In addition, a useful developer for the inventive material is a homogeneous, single part developing agent. The homogeneous, single-part color developing concentrate is prepared using a critical sequence of steps:

In the first step, an aqueous solution of a suitable color developing agent is prepared. This color developing agent is generally in the form of a sulfate salt. Other components of the solution can include an antioxidant for the color developing agent, a suitable number of alkali metal ions (in an at least stoichiometric proportion to the sulfate ions) provided by an alkali metal base, and a photographically inactive water-miscible or water-soluble hydroxy-containing organic solvent. This solvent is present in the final concentrate at a concentration such that the weight ratio of water to the organic solvent is from about 15:85 to about 50:50.

In this environment, especially at high alkalinity, alkali metal ions and sulfate ions form a sulfate salt that is precipitated in the presence of the hydroxy-containing organic solvent. The precipitated sulfate salt can then be readily removed using any suitable liquid/solid phase separation technique (including filtration, centrifugation or decantation). If the antioxidant is a liquid organic compound, two phases may be formed and the precipitate may be removed by discarding the aqueous phase.

The color developing concentrates of this invention include one or more color developing agents that are well known in the art that, in oxidized form, will react with dye forming color couplers in the processed materials. Such color developing agents include, but are not limited to, aminophenols, p-phenylenediamines (especially N,N-dialkyl-p-phenylenediamines) and others which are well known in the art, such as EP 0 434 097 A1 (published Jun. 26, 1991) and EP 0 530 921 A1 (published Mar. 10, 1993). It may be useful for the color developing agents to have one or more water-solubilizing groups as are known in the art. Further details of such materials are provided in *Research*

*Disclosure*, publication 38957, pages 592-639 (September 1996). *Research Disclosure* is a publication of Kenneth Mason Publications Ltd., Dudley House, 12 North Street, Emsworth, Hampshire PO10 7DQ England (also available from Emsworth Design Inc., 121 West 19th Street, New York, N.Y. 10011). This reference will be referred to hereinafter as "Research Disclosure".

Preferred color developing agents include, but are not limited to, N,N-diethyl p-phenylenediamine sulfate (KODAK Color Developing Agent CD-2), 4-amino-3-methyl-N-(2-methane sulfonamidoethyl)aniline sulfate, 4-(N-ethyl-N-β-hydroxyethylamino)-2-methylaniline sulfate (KODAK Color Developing Agent CD-4), p-hydroxyethylaminoaniline sulfate, 4-(N-ethyl-N-2-methanesulfonamidoethyl)-2-methylphenylenediamine sesquisulfate (KODAK Color Developing Agent CD-3), 4-(N-ethyl-N-2-methanesulfonamidoethyl)-2-methylphenylenediamine sesquisulfate, and others readily apparent to one skilled in the art.

In order to protect the color developing agents from oxidation, one or more antioxidants are generally included in the color developing compositions. Either inorganic or organic antioxidants can be used. Many classes of useful antioxidants are known, including but not limited to, sulfites (such as sodium sulfite, potassium sulfite, sodium bisulfite and potassium metabisulfite), hydroxylamine (and derivatives thereof), hydrazines, hydrazides, amino acids, ascorbic acid (and derivatives thereof), hydroxamic acids, aminoketones, mono- and polysaccharides, mono- and polyamines, quaternary ammonium salts, nitroxy radicals, alcohols, and oximes. Also useful as antioxidants are 1,4-cyclohexadienes. Mixtures of compounds from the same or different classes of antioxidants can also be used if desired.

Especially useful antioxidants are hydroxylamine derivatives as described for example, in U.S. Pat. Nos. 4,892,804; 4,876,174; 5,354,646; and 5,660,974, all noted above, and U.S. Pat. No. 5,646,327 (Burns et al). Many of these antioxidants are mono- and dialkylhydroxylamines having one or more substituents on one or both alkyl groups. Particularly useful alkyl substituents include sulfo, carboxy, amino, sulfonamido, carbonamido, hydroxy and other solubilizing substituents.

More preferably, the noted hydroxylamine derivatives can be mono- or dialkylhydroxylamines having one or more hydroxy substituents on the one or more alkyl groups. Representative compounds of this type are described for example in U.S. Pat. No. 5,709,982 (Marrese et al) as having the structure I:



wherein R is hydrogen, a substituted or unsubstituted alkyl group of 1 to 10 carbon atoms, a substituted or unsubstituted hydroxyalkyl group of 1 to 10 carbon atoms, a substituted or unsubstituted cycloalkyl group of 5 to 10 carbon atoms, or a substituted or unsubstituted aryl group having 6 to 10 carbon atoms in the aromatic nucleus.

X<sub>1</sub> is —CR<sub>2</sub>(OH)CHR<sub>1</sub>— and X<sub>2</sub> is —CHR<sub>1</sub>CR<sub>2</sub>(OH)— wherein R<sub>1</sub> and R<sub>2</sub> are independently hydrogen, hydroxy, a substituted or unsubstituted alkyl group of 1 or 2 carbon atoms, a substituted or unsubstituted hydroxyalkyl group of 1 or 2 carbon atoms, or R<sub>1</sub> and R<sub>2</sub> together represent the carbon atoms necessary to complete a substituted or unsubstituted 5- to 8-membered saturated or unsaturated carbocyclic ring structure.

Y is a substituted or unsubstituted alkylene group having at least 4 carbon atoms, and has an even number of carbon atoms, or Y is a substituted or unsubstituted divalent aliphatic group having an even total number of carbon and oxygen atoms in the chain, provided that the aliphatic group has a least 4 atoms in the chain.

Also in Structure I, m, n and p are independently 0 or 1. Preferably, each of m and n is 1, and p is 0.

Specific di-substituted hydroxylamine antioxidants include, but are not limited to: N,N-bis(2,3-dihydroxypropyl)hydroxylamine, N,N-bis(2-methyl-2,3-dihydroxypropyl)hydroxylamine and N,N-bis(1-hydroxymethyl-2-hydroxy-3-phenylpropyl)hydroxylamine. The first compound is preferred.

The colorants can be incorporated into the imaging element by direct addition of the colorant to a coating melt by mixing the colorant with an aqueous medium containing gelatin (or other hydrophilic colloid) at a temperature of 40° C. or higher. The colorant can also be mixed with an aqueous solution of a water-soluble or water-dispersible surfactant or polymer, and passing the premix through a mill until the desired particle size is obtained. The mill can be any high energy device such as a colloid mill, high pressure homogenizer, or the like.

The preferred color of the pigment is blue as a blue pigment incorporated into a gelatin layer offsets the native yellowness of the gelatin yielding a neutral background for the image layers.

Suitable pigments used in this invention can be any inorganic or organic, colored materials which are practically insoluble in the medium in which they are incorporated. The preferred pigments are organic, and are those described in *Industrial Organic Pigments: Production, Properties, Applications* by W. Herbst and K. Hunger, 1993, Wiley Publishers. These include: Azo Pigments such as monoazo yellow and orange, diazo, naphthol, naphthol reds, azo lakes, benzimidazolone, disazo condensation, metal complex, isoindolinone and isoindoline, Polycyclic Pigments such as phthalocyanine, quinacridone, perylene, perinone, diketopyrrolo pyrrole and thiocindigo, and Anthrquinone Pigments such as anthrapyrimidine, flavanthrone, pyranthrone, anthanthrone, dioxazine, triarylcarbodium and quinophthaleone.

The most preferred pigments are the anthraquinones such as Pigment Blue 60, phthalocyanines such as Pigment Blue 15, 15:1, 15:3, 15:4 and 15:6, and quinacridones such as Pigment Red 122, as listed in *NPIRI Raw Materials Data Handbook, Vol. 4, Pigments*, 1983, National Printing Research Institute. These pigments have a dye hue sufficient to overcome the native yellowness of the gelatin imaging layer and are easily dispersed in a aqueous solution.

An aqueous dispersion of the pigments is preferred because the preferred pigments are insoluble in most, if not all, organic solvents, and therefore a high quality dispersion is not likely in a solvent system. In fact, the only solvent that will dissolve preferred pigments PR-122 and PB-15 is concentrated sulfuric acid, which is not an organic solvent. Preferred pigments of the invention are by nature, insoluble, crystalline solids, which is the most thermodynamically stable form that they can assume. In an oil and water dispersion, they would be in the form of an amorphous solid, which is thermodynamically unstable. Therefore, one would have to worry about the pigment eventually converting to the crystalline form with age. We might as well start with a crystalline solid and not worry about preventing the phase transition. Another reason to avoid solvent pigment dispersions is that the high boiling solvent is not removed with

evaporation, and it could cause unwanted interactions in the coating melt such as ripening of DOH dispersion particles, or equilibration with other layers, if it was used in the coating. The use of solid particle dispersion avoids organic solvents altogether.

In the preferred embodiment, the colorant is dispersed in the binder in the form of a solid particle dispersion. Such dispersions are formed by first mixing the colorant with an aqueous solution containing a water-soluble or water-dispersible surfactant or polymer to form a coarse aqueous premix, and adding the premix to a mill. The amount of water-soluble or water-dispersible surfactant or polymer can vary over a wide range, but is generally in the range of 0.01% to 100% by weight of polymer, preferably about 0.3% to about 60%, and more preferably 0.5% to 50%, the percentages being by weight of polymer, based on the weight of the colorant useful in imaging.

The mill can be for example, a ball mill, media mill, attritor mill, vibratory mill or the like. The mill is charged with the appropriate milling media such as, for example, beads of silica, silicon nitride, sand, zirconium oxide, yttria-stabilized zirconium oxide, alumina, titanium, glass, polystyrene, etc. The bead sizes typically range from 0.25 to 3.0 mm in diameter, but smaller media can be used if desired. The premix is milled until the desired particle size range is reached.

The solid colorant particles are subjected to repeated collisions with the milling media, resulting in crystal fracture, deagglomeration, and consequent particle size reduction. The solid particle dispersions of the colorant should have a final average particle size of less than 1 micrometers, preferably less than 0.1 micrometers, and most preferably, the solid colorant particles are of sub-micrometer average size. Solid particle size between 0.01 and 0.1 provides the best pigment utilization and had a reduction in unwanted light absorption compared to pigments with a particle size greater than 1.2 micrometers.

The preferred gelatin to pigment ratio in any gelatin layer is between 65,000:1 to 195,000:1. This gelatin to pigment ratio is preferred as this range provides the necessary color correction to typical photographic imaging layers and typical ink jet dye receiving layers to provide a perceptually preferred neutral background in the image. The preferred coverage of pigment in the gelatin layer is between 0.006 grams/m<sup>2</sup> and 0.020 grams/m<sup>2</sup>. Coverages less than 0.006 gramm/m<sup>2</sup> are not sufficient to provide proper correction of the color and coverages greater than 0.025 grams/m<sup>2</sup> yield a density minimum that has been found to be objectionable by consumers.

Surfactants, polymers, and other additional conventional addenda may also be used in the dispersing process described herein in accordance with prior art solid particle dispersing procedures. Such surfactants, polymers and other addenda are disclosed in U.S. Pat. Nos. 5,468,598; 5,300,394; 5,278,037; 4,006,025; 4,924,916; 4,294,917; 4,940,654; 4,950,586; 4,927,744; 5,279,931; 5,158,863; 5,135,844; 5,091,296; 5,089,380; 5,103,640; 4,990,431; 4,970,139; 5,256,527; 5,089,380; 5,103,640; 4,990,431; 4,970,139; 5,256,527; 5,015,564; 5,008,179; 4,957,857; and 2,870,012, British Patent Specification Nos. 1,570,362 and 1,131,179 referenced above, in the dispersing process of the colorants.

Additional surfactants or other water soluble polymers may be added after formation of the colorant dispersion, before or after subsequent addition of the colorant dispersion to an aqueous coating medium for coating onto an imaging

55

element support. The aqueous medium preferably contains other compounds such as stabilizers and dispersants, for example, additional anionic, nonionic, zwitterionic, or cationic surfactants, and water soluble binders such as gelatin as is well known in the imaging art. The aqueous coating medium may further contain other dispersions or emulsions of compounds useful in imaging.

The following examples illustrate the practice of this invention. They are not intended to be exhaustive of all possible variations of the invention. Parts and percentages are by weight unless otherwise indicated.

## EXAMPLES

### Example 1

In this example a reflective silver halide depth image was created by coating light sensitive silver halide imaging layers on both sides of a flexible, transparent polyester sheet that contained an integral polyethylene layer used to promote silver halide emulsion to the flexible, transparent polymer sheet. After processing the image, the photographic label was laminated to an opaque, white, reflective polypropylene base sheet utilizing a pressure sensitive adhesive. This example will demonstrate a silver halide depth image. Further, this example will show that by printing and developing the duplitized silver halide images on a transparent sheet, improvements in image sharpness and processing efficiency will be obvious.

#### Flexible, Transparent Polyester Sheet:

An oriented polyethylene terephthalate transparent sheet with a thickness of 37 micrometers. The polyethylene terephthalate base had a stiffness of 15 millinewtons in the machine direction and 20 millinewtons in the cross direction. The polyester sheet had an optical transmission of 96%. The transparent polyester sheet had an integral emulsion adhesion layer comprising a low density polyethylene ( $d=0.910 \text{ g/cc}$ ) skin layer on each side that was 1 micrometer thick. The polyethylene skin layers were treated with a corona discharge prior to silver halide coating.

#### Biaxially Oriented Polyolefin Face Stock:

An oriented three layer composite sheet polyolefin sheet (31 micrometers thick) ( $d=0.68 \text{ g/cc}$ ) consisting of a microvoided and oriented polypropylene core (approximately 60% of the total sheet thickness), with a homopolymer non-microvoided oriented polypropylene layer on each side of the voided layer; the void initiating material used was poly(butylene terephthalate). The polypropylene layer adjacent the voided layer contained  $\text{TiO}_2$ , optical brightener, and blue tint to offset the native yellowness of the gelatin used in the silver halide imaging layers.

#### Pressure Sensitive Adhesive:

Permanent Water Based Acrylic Adhesive 12 Micrometers Thick

Silver chloride emulsions were chemically and spectrally sensitized as described below. A biocide comprising a mixture of N-methyl-isothiazolone and N-methyl-5-chloro-isothiazolone was added after sensitization.

#### Blue Sensitive Emulsion (Blue EM-1)

A high chloride silver halide emulsion is precipitated by adding approximately equimolar silver nitrate and sodium chloride solutions into a well-stirred reactor containing glutaryl-diaminophenyl-disulfide, gelatin peptizer, and thioether ripener. Cesium pentachloronitrosylsulfate(II) dopant is added during the silver halide grain formation for most of the precipitation, followed by the addition of potassium hexacyanoruthenate(II), potassium (5-methylthiazole)-

56

pentachloroiridate, a small amount of KI solution, and shelving without any dopant. The resultant emulsion contains cubic shaped grains having edge length of  $0.6 \mu\text{m}$ . The emulsion is optimally sensitized by the addition of a colloidal suspension of aurous sulfide and heat ramped to  $60^\circ \text{C}$ . during which time blue sensitizing dye BSD-4, potassium hexachloroiridate, Lippmann bromide and 1-(3-acetamidophenyl)-5-mercaptopotetrazole were added.

#### Green Sensitive Emulsion (Green EM-1)

A high chloride silver halide emulsion is precipitated by adding approximately equimolar silver nitrate and sodium chloride solutions into a well-stirred reactor containing, gelatin peptizer and thioether ripener. Cesium pentachloronitrosylsulfate(II) dopant is added during the silver halide grain formation for most of the precipitation, followed by the addition of potassium (5-methylthiazole)-pentachloroiridate. The resultant emulsion contains cubic shaped grains of  $0.3 \mu\text{m}$  in edge length size. The emulsion is optimally sensitized by the addition of glutaryl-diaminophenyl-disulfide, a colloidal suspension of aurous sulfide, and heat ramped to  $55^\circ \text{C}$ . during which time potassium hexachloroiridate doped Lippmann bromide, a liquid crystalline suspension of green sensitizing dye GSD-1, and 1-(3-acetamidophenyl)-5-mercaptopotetrazole were added.

#### Red Sensitive Emulsion (Red EM-1)

A high chloride silver halide emulsion is precipitated by adding approximately equimolar silver nitrate and sodium chloride solutions into a well-stirred reactor containing gelatin peptizer and thioether ripener. During the silver halide grain formation, potassium hexacyanoruthenate(II) and potassium (5-methylthiazole)-pentachloroiridate are added. The resultant emulsion contains cubic shaped grains of  $0.4 \mu\text{m}$  in edge length size. The emulsion is optimally sensitized by the addition of glutaryl-diaminophenyl-disulfide, sodium thiosulfate, tripotassium bis{2-[3-(2-sulfobenzamido)phenyl]-mercaptopotetrazole} gold(I) and heat ramped to  $64^\circ \text{C}$ , during which time 1-(3-acetamidophenyl)-5-mercaptopotetrazole, potassium hexachloroiridate, and potassium bromide are added. The emulsion is then cooled to  $40^\circ \text{C}$ , pH adjusted to 6.0 and red sensitizing dye RSD-1 is added.

Coupler dispersions were emulsified by methods well known to the art, and the following layers were coated on the following support:

The following light sensitive silver halide imaging layers were utilized to prepare photographic label utilizing the invention label support material. The following imaging layers were coated utilizing curtain coating:

| Layer   | Item                              | Laydown ( $\text{g/m}^2$ ) |
|---------|-----------------------------------|----------------------------|
| Layer 1 | Blue Sensitive Layer              |                            |
|         | Gelatin                           | 1.3127                     |
|         | Blue sensitive silver (Blue EM-1) | 0.2399                     |
|         | Y-4                               | 0.4143                     |
|         | ST-23                             | 0.4842                     |
|         | Tributyl Citrate                  | 0.2179                     |
|         | ST-24                             | 0.1211                     |
|         | ST-16                             | 0.0095                     |
|         | Sodium Phenylmercaptopotetrazole  | 0.0001                     |
|         | Piperidino hexose reductone       | 0.0024                     |

-continued

| Layer                                | Item                                                                      | Laydown (g/m <sup>2</sup> ) |
|--------------------------------------|---------------------------------------------------------------------------|-----------------------------|
|                                      | 5-chloro-2-methyl-4-isothiazolin-3-one/2-methyl-4-isothiazolin-3-one(3/1) | 0.0002                      |
|                                      | SF-1                                                                      | 0.0366                      |
|                                      | Potassium chloride                                                        | 0.0204                      |
|                                      | Dye-1                                                                     | 0.0148                      |
| <u>Layer 2 Interlayer</u>            |                                                                           |                             |
|                                      | Gelatin                                                                   | 0.7532                      |
|                                      | ST-4                                                                      | 0.1076                      |
|                                      | S-3                                                                       | 0.1969                      |
|                                      | 5-chloro-2-methyl-4-isothiazolin-3-one/2-methyl-4-isothiazolin-3-one(3/1) | 0.0001                      |
|                                      | Catechol disulfonate                                                      | 0.0323                      |
|                                      | SF-1                                                                      | 0.0081                      |
| <u>Layer 3 Green Sensitive Layer</u> |                                                                           |                             |
|                                      | Gelatin                                                                   | 1.1944                      |
|                                      | 1)                                                                        | 0.1011                      |
|                                      | M-4                                                                       | 0.2077                      |
|                                      | Oleyl Alcohol                                                             | 0.2174                      |
|                                      | S-3                                                                       | 0.1119                      |
|                                      | ST-21                                                                     | 0.0398                      |
|                                      | ST-22                                                                     | 0.2841                      |
|                                      | Dye-2                                                                     | 0.0073                      |
|                                      | 5-chloro-2-methyl-4-isothiazolin-3-one/2-methyl-4-isothiazolin-3-one(3/1) | 0.0001                      |
|                                      | SF-1                                                                      | 0.0236                      |
|                                      | Potassium chloride                                                        | 0.0204                      |
|                                      | Sodium Phenylmercaptotetrazole                                            | 0.0007                      |
| <u>Layer 4 M/C Interlayer</u>        |                                                                           |                             |
|                                      | Gelatin                                                                   | 0.7532                      |
|                                      | ST-4                                                                      | 0.1076                      |
|                                      | S-3                                                                       | 0.1969                      |
|                                      | Acrylamide/t-Butylacrylamide sulfonate copolymer                          | 0.0541                      |
|                                      | Bis-vinylsulfonylmethane                                                  | 0.1390                      |
|                                      | 3,5-Dinitrobenzoic acid                                                   | 0.0001                      |
|                                      | Citric acid                                                               | 0.0007                      |
|                                      | Catechol disulfonate                                                      | 0.0323                      |
|                                      | 5-chloro-2-methyl-4-isothiazolin-3-one/2-methyl-4-isothiazolin-3-one(3/1) | 0.0001                      |
| <u>Layer 5 Red Sensitive Layer</u>   |                                                                           |                             |
|                                      | Gelatin                                                                   | 1.3558                      |
|                                      | Red Sensitive silver (Red EM-1)                                           | 0.1883                      |
|                                      | IC-35                                                                     | 0.2324                      |
|                                      | IC-36                                                                     | 0.0258                      |
|                                      | UV-2                                                                      | 0.3551                      |
|                                      | Dibutyl sebacate                                                          | 0.4358                      |
|                                      | S-6                                                                       | 0.1453                      |
|                                      | Dye-3                                                                     | 0.0229                      |
|                                      | Potassium p-toluenethiosulfonate                                          | 0.0026                      |
|                                      | 5-chloro-2-methyl-4-isothiazolin-3-one/2-methyl-4-isothiazolin-3-one(3/1) | 0.0001                      |
|                                      | Sodium Phenylmercaptotetrazole                                            | 0.0005                      |
|                                      | SF-1                                                                      | 0.0524                      |
| <u>Layer 6 UV Overcoat</u>           |                                                                           |                             |
|                                      | Gelatin                                                                   | 0.8231                      |
|                                      | UV-1                                                                      | 0.0355                      |
|                                      | UV-2                                                                      | 0.2034                      |
|                                      | ST-4                                                                      | 0.0655                      |
|                                      | SF-1                                                                      | 0.0125                      |
|                                      | S-6                                                                       | 0.0797                      |
|                                      | 5-chloro-2-methyl-4-isothiazolin-3-one/2-methyl-4-isothiazolin-3-one(3/1) | 0.0001                      |
| <u>Layer 7 SOC</u>                   |                                                                           |                             |
|                                      | Gelatin                                                                   | 0.6456                      |
|                                      | Ludox AM™ (colloidal silica)                                              | 0.1614                      |
|                                      | Polydimethylsiloxane (DC200™)                                             | 0.0202                      |
|                                      | 5-chloro-2-methyl-4-isothiazolin-3-one/2-methyl-4-isothiazolin-3-one(3/1) | 0.0001                      |
|                                      | SF-2                                                                      | 0.0032                      |

-continued

| Layer | Item                          | Laydown (g/m <sup>2</sup> ) |
|-------|-------------------------------|-----------------------------|
| 5     | Tergitol 15-S-5™ (surfactant) | 0.0020                      |
|       | SF-1                          | 0.0081                      |
|       | Aerosol OT™ (surfactant)      | 0.0029                      |

10 The silver halide imaging layers described above were applied to the polyethylene skin layers of the transparent polymer sheet using curtain coating. The silver halide imaging layers were coated at 50% of the grams/m<sup>2</sup> that are listed in the above formulation. The structure of the photographic depth imaging material of the example after application of 15 the silver halide imaging layers is as follows:

|    |                                                                                                                                                                                                                           |
|----|---------------------------------------------------------------------------------------------------------------------------------------------------------------------------------------------------------------------------|
| 20 | Silver halide imaging layers of the example<br>Oriented polyethylene (1 micrometer)<br>Oriented polyester 96% optical transmission<br>Oriented polyethylene (1 micrometer)<br>Silver halide imaging layers of the example |
|----|---------------------------------------------------------------------------------------------------------------------------------------------------------------------------------------------------------------------------|

25 The 10 mm slit rolls of light sensitive silver halide emulsion coated depth imaging material of this example were printed using a digital CRT photographic printer. Several test images were printed on the photographic label material. The printed images were then developed using standard reflective RA4 photographic wet chemistry. At this point, the developed silver halide image was formed on a thin transparent support. To create a reflective depth image, the printed developed imaging layers coated on the transparent polyester sheet were then laminated to the opaque, white reflective biaxially oriented polyolefin sheet utilizing 30 an acrylic pressure sensitive adhesive. The following was the structure of the laminated depth imaging element of the example:

|    |                                                                                                                                                                                                                                                                                                                                                  |
|----|--------------------------------------------------------------------------------------------------------------------------------------------------------------------------------------------------------------------------------------------------------------------------------------------------------------------------------------------------|
| 40 | Developed silver halide imaging layers<br>Oriented polyethylene (1 micrometer)<br>Oriented polyester<br>Oriented polyethylene (1 micrometer)<br>Developed silver halide imaging layers<br>Acrylic pressure sensitive adhesive<br>Polypropylene with blue tint and 14% rutile TiO <sub>2</sub><br>Oriented, voided polypropylene<br>Polypropylene |
|----|--------------------------------------------------------------------------------------------------------------------------------------------------------------------------------------------------------------------------------------------------------------------------------------------------------------------------------------------------|

50 The color photographic reflective depth image laminated to the biaxially oriented base of this invention created a perceptually preferred sense of depth compared to prior art color reflective images. The silver halide imaging layers were simultaneously exposed and, therefore, were in register 55 adding to the quality of the depth image. Because the two silver halide images were in register and were separated by a transparent sheet, the image appears to have depth, better representing the real subject more realistically.

Additionally, the elements of the invention are lighter in 60 weight and thickness compared to prior art photographic paper. A roll of light sensitive silver halide coated thin biaxially oriented sheets of the same diameter will contain 800% more images per printed roll compared to thick prior art photographic paper reducing the manufacturing cost of 65 depth imaging material. Further, because the imaging materials of the invention are light and thin, they can be mailed at a much lower cost compared to prior art photographic

paper. Because the silver halide imaging layers coated on each side of the transparent polyester contained approximately 50% less coverage than prior art photographic papers, the image development was reduced from 45 seconds to 23 seconds without any loss in image quality.

The photographic elements of the invention also are less susceptible to curl, as 50% of the typical amount of gelatin is sealed from humidity contamination to a great degree. Finally, during the printing process, exceptional image sharpness was observed which contributed to the detail and quality of the depth image. Because the invention was printed without a cellulose paper base common to prior art photographic papers, the unwanted secondary exposure that occurs when light energy is scattered by the paper fibers and  $TiO_2$  was avoided.

The invention has been described in detail with particular reference to certain preferred embodiments thereof, but it will be understood that variations and modifications can be effected within the spirit and scope of the invention.

What is claimed is:

1. A photographic element comprising a transparent sheet having a developed photographic image on each side, adhesively connected to a reflective base wherein the photographic image on each side of said transparent sheet comprises an image consisting of magenta, cyan, and yellow dye.

2. The photographic element of claim 1 wherein magenta, yellow, and cyan dye density on each side of said transparent sheet varies by no more than 10 percent.

3. The photographic element of claim 1 wherein said base comprises at least one voided biaxially oriented polyolefin sheet.

4. The photographic element of claim 1 wherein said base comprises at least one voided biaxially oriented polymer sheet.

5. The photographic element of claim 1 wherein said base has a percent reflection of greater than 90 percent across the visible spectrum of between 400 and 700 nm.

6. The photographic element of claim 1 wherein said base comprises a reflective metallic surface.

7. The photographic element of claim 1 wherein said base is retro reflective.

8. The photographic element of claim 1 wherein said base has an  $L^*$  of at least 93.5.

9. The photographic element of claim 1 wherein said base has a percent of transmission no greater than 10 percent.

10. The photographic element of claim 1 wherein a substantially clear layer of adhesive material adhesively connects said base and said transparent sheet having a photographically developed image on each side.

11. The photographic element of claim 10 wherein said adhesive material has a thickness of between 2 and 40 micrometers.

12. The photographic element of claim 10 wherein said adhesive material comprises an acrylic pressure sensitive adhesive.

13. The photographic element of claim 1 wherein said transparent sheet has a thickness of between 6 and 100 micrometers.

14. The photographic element of claim 1 wherein said transparent sheet has a ratio of thickness in micrometers to index of refraction of between 4 and 55.

15. The photographic element of claim 1 wherein said transparent sheet comprises a polymer.

16. The photographic element of claim 1 wherein said transparent sheet comprises a biaxially oriented polyolefin sheet or oriented polyester sheet.

17. The photographic element of claim 1 wherein said transparent sheet has an emulsion adhesion layer.

18. The photographic element of claim 1 wherein said transparent sheet has at least one surface that has functional end group chemistry on the surface.

19. The photographic element of claim 1 wherein said transparent sheet has an integral layer of polyethylene on at least one surface.

20. The photographic element of claim 1 wherein said magenta, yellow, and cyan dyes are each present in substantially equal amounts on each side of said transparent sheet.

21. A method of forming a photographic image comprising providing a transparent sheet having at least one photosensitive silver halide layer on each side, exposing said at least one photosensitive silver halide layer on each side to actinic radiation, and developing the silver halide to form an image, bringing the transparent sheet having developed images thereon into adhesive contact with a reflective base.

22. The method of claim 21 wherein adhesive contact is achieved by coating an adhesive material on said reflective base prior to bringing into contact with said transparent sheet having developed images thereon.

23. The method of claim 21 wherein adhesive contact is achieved by coating an adhesive material on said transparent sheet having developed images thereon prior to bringing into contact with said base.

24. The method of claim 21 wherein said exposing is by a scanning collimated beam.

25. The method of claim 21 wherein said exposing is by a negative working optical exposure.

26. The method of claim 21 wherein said exposing is by a cathode ray tube.

27. The method of claim 21 wherein the developed photographic image on each side of said transparent sheet comprises an image consisting of magenta, cyan, and yellow dye.

28. The method of claim 21 wherein said base comprises at least one voided biaxially oriented polyolefin sheet.

29. The method of claim 21 wherein said base comprises at least one voided biaxially oriented polymer sheet.

30. The method of claim 21 wherein said transparent sheet has a ratio of thickness in micrometers to index of refraction of between 4 and 55.

31. The method of claim 27 wherein said transparent sheet has at least one surface that has functional end group chemistry on the surface.

32. The method of claim 27 wherein said magenta, yellow, and cyan dye density on each side of said transparent sheet varies by between 15 and 60 percent.

33. A photographic element comprising a transparent sheet having a developed photographic image on each side, adhesively connected to a reflective base, wherein said base comprises at least one voided biaxially oriented polymer sheet.

34. The photographic element of claim 33 wherein said base comprises at least one voided biaxially oriented polyolefin sheet.

35. The photographic element of claim 33 wherein said base has a percent reflection of greater than 90 percent across the visible spectrum of between 400 and 700 nm.

36. The photographic element of claim 35 wherein the photographic image on each side of said transparent sheet comprises an image consisting of magenta, cyan, and yellow dye.

37. The photographic element of claim 33 wherein said base comprises a reflective metallic surface.

38. The photographic element of claim 33 wherein said base is retro reflective.

**61**

**39.** The photographic element of claim **33** wherein said base has a percent of transmission no greater than 10 percent.

**40.** The photographic element of claim **33** wherein said transparent sheet has a thickness of between 6 and 100 micrometers.

**41.** The photographic element of claim **33** wherein said transparent sheet comprises an oriented polyester sheet.

**42.** The photographic element of claim **33** wherein said transparent sheet has at least one surface that has functional end group chemistry on the surface.

**43.** The photographic element of claim **33** wherein said transparent sheet has an integral layer of polyethylene on at least one surface.

**44.** The photographic element of claim **33** wherein said magenta, yellow, and cyan dye density on each side of said transparent sheet varies by between 15 and 60 percent.

**45.** The photographic element of claim **28** wherein the photographic image on each side of said transparent sheet comprises metallic silver.

**46.** A photographic element comprising a transparent sheet having a developed photographic image on each side, adhesively connected to a reflective base wherein said transparent sheet has at least one surface that has functional end group chemistry on the surface.

**47.** The photographic element of claim **46** wherein said transparent sheet has a thickness of between 6 and 100 micrometers.

**48.** The photographic element of claim **46** wherein said transparent sheet has a ratio of thickness in micrometers to index of refraction of between 4 and 55.

**49.** The photographic element of claim **47** wherein the photographic image on each side of said transparent sheet comprises an image consisting of magenta, cyan, and yellow dye.

**50.** The photographic element of claim **48** wherein said base comprises at least one voided biaxially oriented polyolefin sheet.

**62**

**51.** The photographic element of claim **46** wherein said base comprises at least one voided biaxially oriented polymer sheet.

**52.** The photographic element of claim **46** wherein said base comprises a reflective metallic surface.

**53.** The photographic element of claim **46** wherein said transparent sheet has an integral layer of polyethylene on at least one surface.

**54.** The photographic element of claim **49** wherein said magenta, yellow, and cyan dyes are each present in substantially equal amounts on each side of said transparent sheet.

**55.** The photographic element of claim **49** wherein magenta, yellow, and cyan dye density on each side of said transparent sheet varies by no more than 10 percent.

**56.** The photographic element of claim **49** wherein said magenta, yellow, and cyan dye density on each side of said transparent sheet varies by between 15 and 60 percent.

**57.** The photographic element of claim **46** wherein the photographic image on each side of said transparent sheet comprises metallic silver.

**58.** A photographic element comprising a transparent sheet having a developed photographic image on each side, adhesively connected to a reflective base wherein the photographic image on each side of said transparent sheet comprises an image consisting of magenta, cyan, and yellow dye, and said magenta, yellow, and cyan dye density on each side of said transparent sheet varies by between 15 and 60 percent.

**59.** The photographic element of claim **58** wherein said base comprises at least one voided biaxially oriented polymer sheet.

**60.** The photographic element of claim **58** wherein said transparent sheet comprises an oriented polyester sheet.

**61.** The photographic element of claim **58** wherein said transparent sheet has at least one surface that has functional end group chemistry on the surface.

\* \* \* \* \*